# EUROPEAN PATENT SPECIFICATION

(11) **EP 4 284 902 B1**
(45) Date of publication and mention of the grant of the patent: **20.08.2025**
(21) Application number: 22700409.0
(22) Date of filing: 17.01.2022
(51) Int. Cl.: C10L 1/222, C10L 10/00, C10L 10/04, C10L 10/06, C10L 1/02

(54) **BRANCHED PRIMARY ALKYL AMINES AS ADDITIVES FOR GASOLINE FUELS**
VERZWEIGTE PRIMÄRE ALKYLAMINE ALS ADDITIVE FÜR BENZINKRAFTSTOFFE
ALKYLAMINES PRIMAIRES RAMIFIÉES EN TANT QU'ADDITIFS POUR CARBURANTS À BASE D'ESSENCE

(30) Priority: 27.01.2021 EP 21153753
(43) Date of publication of application: 06.12.2023
(73) Proprietor: BASF SE, 67056 Ludwigshafen am Rhein (DE)
(72) Inventor: MEZGER, Jochen, 67056 Ludwigshafen (DE); WALTER, Marc, 67056 Ludwigshafen (DE); HANSCH, Markus, 67056 Ludwigshafen (DE); CSIHONY, Szilard, 69517 Gorxheimertal (DE); LOHMANN, Mathias, 67056 Ludwigshafen (DE)
(74) Representative: BASF IP Association
(86) International application number: PCT/EP2022/050862
(87) International publication number: WO 2022/161803

(56) References cited:
- EP-B1- 2 855 642
- AU-B2- 509 125
- CA-A- 781 869
- US-A1- 2005 172 545

## Description

The present invention describes the use of certain branched amines as additives for unleaded gasoline fuels, especially for reducing injector nozzle fouling in direct injection spark ignition engines. The use of linear amines as additives for different fuels and for different purposes is long known.

EP 450704 discloses linear C₁₀- to C₂₀-amines as additives for reducing fouling of injectors in Diesel engines.

WO 2003/76554 discloses the use of hydrocarbyl amines wherein the hydrocarbyl moiety has a number average molecular weight in the range 140 to 255 as an additive for reducing injector nozzle fouling in a direct injection spark ignition engine.

Linear alkylamines are preferred, in the examples dodecyl amine (lauryl amine) was used.

WO 2004/50806 A2 discloses a composition comprising amines and Mannich adducts as detergent for direct injection spark ignition engines.

Among other amines *inter alia* tridecyl amine is generically disclosed and used in one additive package without disclosing which isomer was used.

It is a disadvantage of linear amines that they tend to solidify at ambient temperatures so that incorporation of linear amines into additive packages requires a minimum temperature or heating of the components before mixing. Especially lauryl amine, as disclosed in WO 2003/76554, is solid a room temperature and therefore needs to be molten before formulating an additive package. Furthermore, additive packages comprising lauryl amine as constituent show poor storage stability at low temperatures (see Comparative Examples below).

Furthermore, linear amines tend to demix from additive packages so that a higher amount of solvent or a stabiliser or compatibilizer is to be used as an additional component in order to yield stable mixtures.

It was an object of the present invention to develop amines as additives for unleaded gasoline fuels which exhibit an activity as an additive for reducing injector nozzle fouling comparable to the linear amines known from the prior art or even a higher activity but do not show their disadvantages but are easier to incorporate into an additive package. Furthermore, the storage stability of the amine-containing additive packages should be improved.

The problem was solved by the use of branched alkyl amine R-NH₂, the alkyl group R having from 8 to 22, preferably from 10 to 17, more preferably 13 carbon atoms and with a branching of at least 1.0, preferably of from 1.0 to 8.0, more preferably from 1.5 to 7.0 as a fuel additive in unleaded gasoline.

Another object of the present invention are unleaded gasoline additive packages comprising at least one of these branched alkyl amines, at least one deposit control agent, and optionally further gasoline additives.

Another object of the present invention are unleaded gasoline fuel compositions comprising such additive packages. Such unleaded gasoline fuel compositions are preferably suitable for use in a spark ignition engine, for reducing injector nozzle fouling in a direct injection spark ignition engine.

Therefore, further object of the present invention are the use of branched primary alkyl amines R-NH₂, the alkyl group R having from 8 to 22, preferably from 10 to 17, more preferably 13 carbon atoms and with a branching of at least 1.0, preferably of from 1.0 to 8.0, more preferably from 1.5 to 7.0 for reducing injector nozzle fouling in a direct injection spark ignition engine, the use of additive packages comprising such branched primary alkyl amines for reducing injector nozzle fouling in a direct injection spark ignition engine, and the use of an unleaded gasoline composition comprising a major proportion of a gasoline suitable for use in a spark ignition engine, for reducing injector nozzle fouling in a direct injection spark ignition engine.

### Branched Amine

The branched alkyl amines R-NH₂ according to the present invention are primary amines bearing an alkyl group R having from 8 to 22, preferably from 10 to 17, more preferably 13 carbon atoms, the alkyl group having a branching of at least 1.0, preferably of from 1.0 to 8.0, more preferably from 1.5 to 7.0.

"Branching" in the context of the present invention means that the alkyl residue R comprises the required number of branchings. In the case of a single amine with only one branched isomer the branching of that pure compound can be easily determined on the basis of the chemical structure. In case of isomer mixtures the average branching of the mixture is calculated by adding up the branching of each individual isomer multiplied by the molar amount of the respective isomer in the mixture. Preferably, the branching is determined using the branching index (ISO index) (see below).

The branched primary amines can be used as a mixture of amines of different molecular weight or preferably of one single molecular weight.

Typical examples of such amines are the branched isomers of octyl amine, nonyl amine, decyl amine, undecyl amine, dodecyl amine, tridecyl amine, tetradecyl amine, pentadecyl amine, hexadecyl amine, and heptadecyl amine, preferably nonyl amine, decyl amine, dodecyl amine, tridecyl amine, tetradecyl amine, hexadecyl amine, heptadecyl amine, eicosyl amine, docosyl amine, and mixtures thereof, more preferably nonyl amine, tridecyl amine, and heptadecyl amine, most preferably tridecyl amine and heptadecyl amine, and especially tridecyl amine. One preferred example for a branched octyl amine is 2-amino-2,4,4-trimethyl-pentane.

One preferred example for a branched decyl amine is 2-propylheptyl amine.

In a preferred embodiment the branched amines according to the present invention are obtainable by oligomerization of propene, isobutene, 1-butene or 2-butene forming a double bond-containing oligomer, followed by hydroformylation and reductive amination with ammonia. The resulting amine usually is a mixture of isomers.

In another preferred embodiment the branched amines according to the present invention are obtainable by amination of the corresponding branched alcohols or by reductive amination of the corresponding branched aldehydes. In this case the branching of the amines obtained is the same as that of the underlying alcohols or aldehydes, since the reaction conditions of the amination or reductive amination usually do not affect the branching of the alkyl group.

In the case of the branched tridecyl amine the mixture of isomers my contain one or more of the following isomers:
2,2,4,4,6,6-Hexa methyl heptyl amine, 2,4,6-tri ethyl heptyl amine, 2,3,4,5,6-penta methyl octyl amine, heptyl amines bearing 2 ethyl groups and 2 methyl groups in position 2, 4, and 6, and heptyl amines bearing 1 ethyl group and 4 methyl groups in position 2, 4, and 6.

Isomer mixtures with 2,2,4,4,6,6-hexa methyl heptyl amine or 2,4,6-tri ethyl heptyl amine as main constituents are most preferred.

Examples of mixtures of such branched amines are mixtures of tertiary alkyl C₁₂- to C₁₄-amines (CAS No 68955-53-3) or of C₁₆- to C₂₂-amines obtainable via Ritter reaction.

Amines with tertiary alkyl groups are less preferred since they exhibit a toxicity on inhalation. Hence, among the branched primary alkyl amines according to the invention those amines with the amine group bound to a primary carbon are preferred, i.e. amines bearing a group -CH₂-NH₂.

Especially preferred is a tridecylamine isomeric mixture from BASF SE (CAS No: 86089-17-0) obtained by amination from the corresponding tridecanol isomeric mixture with a branching index of 2.2.

Such branched alkyl amines exhibit a lower melting point than the corresponding linear alkyl amines and are, therefore, easier to formulate in additive packages. Often such branched alkyl amines are liquid at room temperature, however, usually exhibit a lower melting point than the corresponding linear isomers. With easier formulability is meant that less solvent is needed to achieve a homogenous formulation compared to the corresponding linear alkyl amines.

Therefore, it is an object of the present invention to use such branched primary alkyl amines R-NH₂, the alkyl group R having from 8 to 22, preferably from 10 to 17, more preferably 13 carbon atoms and with a branching of at least 1.0, preferably of from 1.0 to 8.0, more preferably from 1.5 to 7.0 as an additive in a fuel additive package for improving the storage stability and/or formulability of fuel additive packages comprising
- at least one deposit control agent selected from the group consisting of
   -- quaternary ammonium compounds,
   -- Mannich adducts, and
   -- polyalkenemono- or polyalkenepolyamines having a number average molecular weight in the range 300 to 5000, and
- optionally at least one further gasoline fuel additive, selected from the group consisting of
   -- friction modifiers,
   -- dehazers,
   -- antioxidants,
   -- metal deactivators,
   -- corrosion inhibitors,
   -- carrier oils, and
   -- solvents
for unleaded gasoline compositions suitable for use in a spark ignition engine, for reducing injector nozzle fouling in a direct injection spark ignition engine.

### Branching index (ISO index)

According to the invention the degree of branching is preferably described by the ISO index which indicates the average number of branches of the respective alkyl groups. Thus, for example, in the case of a C₈ alkyl group, the n-octyl group contributes 0, methylheptyl groups contribute 1, and dimethylhexyl groups contribute 2 to the ISO index. The lower the ISO index, the greater the linearity of the molecules in the respective group.

The degree of branching is defined as the number of methyl groups in a molecule of the amine minus 1. The average degree of branching is the statistical average of the degree of branching of the molecules of a sample. The average degree of branching can be preferably determined by ¹H-NMR spectroscopy as follows: a sample of the amine is firstly subject to derivatization by means of trichloroacetyl isocyanate (TAI) (literature: A. K. Bose, P. R. Srinivasan, Tetrahedron 1975, 3025; A. Postma et al., Polymer 2006, 1899). The signals of the methylene group adjacent to the amino group are at δ = 3 to 4 ppm. All methyl, methylene and methine protons are in the range from 2.4 to 0.4 ppm. The signals < 1 ppm are assigned to the methyl groups. The average degree of branching (ISO index) can be calculated as follows from the spectrum obtained in this way: $ISO index = \left(\left(A\left({CH}_{3}\right)/3\right)/\left(A\left({CH}_{2}-{NH}_{2}\right)/2\right)\right) - 1$ where A(CH₃) is the signal area corresponding to the methyl protons and A(CH₂-NH₂) is the signal area of the methylene protons in the CH₂-NH₂ group. Primary amines bearing methine protons adjacent to the amino group (H₂NCHR) may be analysed analogously. In the case of amines bearing a quaternary carbon atom adjacent to the amino group another distinct and assignable proton signal may be used for determining the ISO index.

In the case of branched amines obtained from the corresponding branched alcohols or aldehydes by amination or reductive amination the ISO index determined according to the above-mentioned method may be used.

An even more preferred ¹H-NMR method is handled without derivatization: The degree of branching (ISO index) of primary amines with no α-branching (H₂NCH₂R) is determined from their ¹H-NMR spectra. All NMR spectra were recorded at T = 298.2 K on a Bruker Avance III 400 spectrometer operating at 400.33 MHz for ¹H and 100.66 MHz for ¹³C. The spectrometer was equipped with a 5 mm z-gradient broadband observe smartprobe. Chemical shifts are referenced to Tetramethylsilane (TMS, δ(TMS) = 0 ppm). 1H 1D spectra were recorded using the zg pulse program with 64k data points, the relaxation delay D1 was chosen as 5 seconds, and 64 transients were recorded. For processing in Bruker TopSpin 4.0.9 software, 32k data points were used, an exponential window function with a line broadening of 0.3 Hz was applied. Automatic baseline correction was used, phase correction was performed manually by the user. Phase sensitive HSQC spectra were recorded using the hsqcedetgpsisp2.3 pulse sequence, with 4k data points in the direct and 256 data points in the indirect dimension using 8 transients per increment. Experiments were optimized for a ¹J_{C-H} coupling constant of 144 Hz. The relaxation delay D1 was set to 1.0 s. For processing, 1024 x 1024 data points were Fourier transformed, and a quadratic sine function with a sine bell shift of 2 was applied.

Samples were prepared by dissolution of the pure analyte in deuterated chloroform with traces of TMS as internal reference. The samples were transferred into 5 mm NMR tubes. Deuterated solvents were purchased from Euriso-Top GmbH and used as received.

For the determination of the ISO index, the integral for H₂NCH₂R from δ = 2.3 - 2.95 ppm is set to a value of 2. The signals of the aliphatic methyl groups (verified by phase-sensitive HSQC spectroscopy) are integrated from δ = 0.6 - 0.95 ppm giving the value I(Me). The degree of branching (ISO index) is calculated according to ISO index = I(Me)/3 -1.

### Deposit control agent

The unleaded gasoline additive packages respectively unleaded gasoline compositions according to the present invention comprise at least one deposit control agent, selected from the group consisting of
- quaternary ammonium compounds,
- Mannich adducts, and
- polyalkenemono- or polyalkenepolyamines having a number average molecular weight in the range 300 to 5000,
   preferably selected from the group consisting of
- quaternary ammonium compounds, and
- polyalkenemono- or polyalkenepolyamines having a number average molecular weight in the range 300 to 5000.

Most preferably the deposit control agent is a polyalkenemono- or polyalkenepolyamines, especially a polyisobutene amine having a number average molecular weight in the range 300 to 5000.

The deposit control agents are described in more detail below:

### Quaternary ammonium compounds

The at least one quaternary nitrogen component refer, in the context of the present invention, to nitrogen compounds quaternized in the presence of an acid or in an acid-free manner, preferably obtainable by addition of a compound comprising at least one oxygen- or nitrogen-containing group reactive with an anhydride and additionally at least one quaternizable amino group onto a polycarboxylic anhydride compound and subsequent quaternization.

In most cases the quaternary nitrogen component is an ammonium compound, however in the context of the present document morpholinium, piperidinium, piperazinium, pyrrolidinium, imidazolinium or pyridinium cations are also encompassed by the phrase "quaternary nitrogen component".

The quaternary ammonium compounds are preferably of the formula

⁺NR¹R²R³R⁴ A⁻

in which
A⁻ stands for an anion, preferably a carboxylate R⁵COO⁻ or a carbonate R⁵O-COO⁻,
   and
R¹, R², R³, R⁴, and R⁵ independently of another are an organic residue with from 1 to 100 carbon atoms, substituted or unsubstituted, preferably unsubstituted, linear or branched alkyl, alkenyl or hydroxyalkyl residue with 1 to 100, more preferably 1 to 75, even more preferably 1 to 30, most preferably 1 to 25 and especially 1 to 20 carbon atoms,
R⁵ additionally may be substituted or unsubstituted cycloalkyl or aryl residues bearing 5 to 20, preferably 5 to 12 carbon atoms.

It is also possible that the anion may be multiply charged negatively, e.g. if anions of dibasic acids are used, in this case the stoichiometric ratio of the ammonium ions to the anions corresponds to the ratio of positive and negative charges.

The same is true for salts in which the cation bears more than one ammonium ion, e.g. of the substituents connect two or more ammonium ions.

In the organic residues the carbon atoms may be interrupted by one or more oxygen and/or sulphur atoms and/or one or more substituted or unsubstituted imino groups, and may be substituted by C₆-C₁₂-aryl, C₅-C₁₂-cycloalkyl or a five- or six-membered, oxygen-, nitrogen- and/or sulphur-containing heterocycle or two of them together form an unsaturated, saturated or aromatic ring which may be interrupted by one or more oxygen and/or sulphur atoms and/or one or more substituted or unsubstituted imino groups, where the radicals mentioned may each be substituted by functional groups, aryl, alkyl, aryloxy, alkyloxy, halogen, heteroatoms and/or heterocycles.

Two of the residues R¹ to R⁴ may together form an unsaturated, saturated or aromatic ring, preferably a five-, six- or seven-membered ring (including the nitrogen atom of the ammonium ion).

In this case the ammonium cation may be a morpholinium, piperidinium, piperazinium, pyrrolidinium, imidazolinium or pyridinium cation.

In these definitions
C₁-C₂₀-alkyl which may be substituted by functional groups, aryl, alkyl, aryloxy, alkyloxy, halogen, heteroatoms and/or heterocycles is, for example, methyl, ethyl, propyl, isopropyl, n-butyl, sec-butyl, tert-butyl, pentyl, hexyl, heptyl, octyl, 2-ethylhexyl, 2,4,4-trimethylpentyl, decyl, dodecyl, tetradecyl, heptadecyl, octadecyl, eicosyl, 1,1-dimethylpropyl, 1,1-dimethylbutyl, 1,1,3,3-tetramethylbutyl, benzyl, 1-phenylethyl, 2-phenylethyl, α,α-dimethylbenzyl, benzhydryl, p-tolylmethyl,1-(p-butylphenyl)ethyl, p-chlorobenzyl, 2,4-dichlorobenzyl, p-methoxybenzyl, methoxybenzyl, 2-cyanoethyl, 2-cyanopropyl, 2-methoxycarbonylethyl, 2-ethoxycarbonylethyl, 2-butoxycarbonylpropyl, 1,2-di-(methoxycarbonyl)ethyl, 2-methoxyethyl, 2-ethoxyethyl, 2-butoxyethyl, diethoxymethyl, diethoxyethyl, 1,3-dioxolan-2-yl, 1,3-dioxan-2-yl, 2-methyl-1,3-dioxolan-2-yl, 4-methyl-1,3-dioxolan-2-yl, 2-isopropoxyethyl, 2-butoxypropyl, 2-octyloxyethyl, chloromethyl, 2-chloroethyl, trichloromethyl, trifluoromethyl, 1,1-dimethyl-2-chloroethyl, 2-methoxyisopropyl, 2-ethoxyethyl, butylthiomethyl, 2-dodecylthioethyl, 2-phenylthioethyl, 2,2,2-trifluoroethyl, 2-hydroxyethyl, 2-hydroxypropyl, 3-hydroxypropyl, 4-hydroxybutyl, 6-hydroxyhexyl, 2-aminoethyl, 2-aminopropyl, 3-aminopropyl, 4-aminobutyl, 6-aminohexyl, 2-methylaminoethyl, 2-methylaminopropyl, 3-methylaminopropyl, 4-methylaminobutyl, 6-methylaminohexyl, 2-dimethylaminoethyl, 2-dimethylaminopropyl, 3-dimethylaminopropyl, 4-dimethylaminobutyl, 6-dimethylaminohexyl, 2-hydroxy-2,2-dimethylethyl, 2-phenoxyethyl, 2-phenoxypropyl, 3-phenoxypropyl, 4-phenoxybutyl, 6-phenoxyhexyl, 2-methoxyethyl, 2-methoxypropyl, 3-methoxypropyl, 4-methoxybutyl, 6-methoxyhexyl, 2-ethoxyethyl, 2-ethoxypropyl, 3-ethoxypropyl, 4-ethoxybutyl or 6-ethoxyhexyl, and
C₂-C₂₀-alkyl interrupted by one or more oxygen and/or sulphur atoms and/or one or more substituted or unsubstituted imino groups is, for example, 5-hydroxy-3-oxa-pentyl, 8-hydroxy-3,6-dioxaoctyl, 11-hydroxy-3,6,9-trioxaundecyl, 7-hydroxy-4-oxaheptyl, 11-hydroxy-4,8-dioxaundecyl, 15-hydroxy-4,8,12-trioxapentadecyl, 9-hydroxy-5-oxanonyl, 14-hydroxy-5,10-oxatetradecyl, 5-methoxy-3-oxapentyl, 8-methoxy-3,6-dioxaoctyl, 11-methoxy-3,6,9-trioxaundecyl, 7-methoxy-4-oxaheptyl, 11-methoxy-4,8-dioxa-undecyl, 15-methoxy-4,8,12-trioxapentadecyl, 9-methoxy-5-oxanonyl, 14-methoxy-5,10-oxatetradecyl, 5-ethoxy-3-oxapentyl, 8-ethoxy-3,6-dioxaoctyl, 11-ethoxy-3,6,9-trioxaundecyl, 7-ethoxy-4-oxaheptyl, 11-ethoxy-4,8-dioxaundecyl, 15-ethoxy-4,8,12-trioxapentadecyl, 9-ethoxy-5-oxanonyl or 14-ethoxy-5,10-oxatetradecyl.

If two radicals form a ring, they can together be 1,3-propylene, 1,4-butylene, 1,5-pentylene, 2-oxa-1,3-propylene, 1-oxa-1,3-propylene, 2-oxa-1,3-propylene, 1-oxa-1,3-propenylene, 1-aza-1,3-propenylene, 1-C₁-C₄-alkyl-1-aza-1,3-propenylene, 1,4-buta-1,3-dienylene, 1-aza-1,4-buta-1,3-dienylene or 2-aza-1,4-buta-1,3-dienylene.

The number of oxygen and/or sulphur atoms and/or imino groups is not subject to any restrictions. In general, there will be no more than 5 in the radical, preferably no more than 4 and very particularly preferably no more than 3.

Furthermore, there is generally at least one carbon atom, preferably at least two carbon atoms, between any two heteroatoms.

Substituted and unsubstituted imino groups can be, for example, imino, methylimino, isopropy-limino, n-butylimino or tert-butylimino.

Furthermore,
functional groups can be carboxy, carboxamide, hydroxy, di(C₁-C₄-alkyl)amino, C₁-C₄-alkyloxycarbonyl, cyano or C₁-C₄-alkyloxy,
C₆-C₁₂-aryl which may be substituted by functional groups, aryl, alkyl, aryloxy, alkyloxy, halogen, heteroatoms and/or heterocycles is, for example, phenyl, tolyl, xylyl, α-naphthyl, β-naphthyl, 4-diphenylyl, chlorophenyl, dichlorophenyl, trichlorophenyl, difluorophenyl, methylphenyl, dimethylphenyl, trimethylphenyl, ethylphenyl, diethylphenyl, isopropylphenyl, tert-butylphenyl, dodecylphenyl, methoxyphenyl, dimethoxyphenyl, ethoxyphenyl, hexyloxyphenyl, methylnaphthyl, isopropylnaphthyl, chloronaphthyl, ethoxynaphthyl, 2,6-dimethylphenyl, 2,4,6-trimethylphenyl, 2,6-dimethoxyphenyl, 2,6-dichlorophenyl, 4-bromophenyl, 2- or 4-nitrophenyl, 2,4- or 2,6-dinitrophenyl, 4-dimethylaminophenyl, 4-acetylphenyl, methoxyethylphenyl or ethox-ymethylphenyl,
C₅-C₁₂-cycloalkyl which may be substituted by functional groups, aryl, alkyl, aryloxy, alkyloxy, halogen, heteroatoms and/or heterocycles is, for example, cyclopentyl, cyclohexyl, cyclooctyl, cyclododecyl, methylcyclopentyl, dimethylcyclopentyl, methylcyclohexyl, dimethylcyclohexyl, diethylcyclohexyl, butylcyclohexyl, methoxycyclohexyl, dimethoxycyclohexyl, diethoxycyclohex-yl, butylthiocyclohexyl, chlorocyclohexyl, dichlorocyclohexyl, dichlorocyclopentyl or a saturated or unsaturated bicyclic system such as norbornyl or norbornenyl,
a five- or six-membered, oxygen-, nitrogen- and/or sulphur-containing heterocycle is, for example, furyl, thienyl, pyrryl, pyridyl, indolyl, benzoxazolyl, dioxolyl, dioxyl, benzimidazolyl, benzothiazolyl, dimethylpyridyl, methylquinolyl, dimethylpyrryl, methoxyfuryl, dimethoxypyridyl, difluoro-pyridyl, methylthienyl, isopropylthienyl or tert-butylthienyl and
C₁ to C₄-alkyl is, for example, methyl, ethyl, propyl, isopropyl, n-butyl, sec-butyl or tert-butyl.

The residues R¹ to R⁵ are preferably C₂-C₁₈-alkyl or C₆-C₁₂-aryl, more preferably C₄-C₁₆-alkyl or C₆-C₁₂-aryl, and even more preferably C₄-C₁₆-alkyl or C₆-aryl.

The residues R¹ to R⁵ may be saturated or unsaturated, preferably saturated.

Preferred residues R¹ to R⁵ do not bear any heteroatoms other than carbon or hydrogen.

Preferred examples of R¹ to R⁴ are methyl, ethyl, propyl, isopropyl, n-butyl, sec-butyl, tert-butyl, pentyl, hexyl, heptyl, octyl, 2-ethylhexyl, 2,4,4-trimethylpentyl, 2-propylheptyl, decyl, dodecyl, tetradecyl, heptadecyl, octadecyl, eicosyl, 1,1-dimethylpropyl, 1,1-dimethylbutyl, 1,1,3,3-tetramethylbutyl, benzyl, 1-phenylethyl, 2-phenylethyl, α,α-dimethylbenzyl, benzhydryl, p-tolylmethyl or 1-(p-butylphenyl)ethyl.

In a preferred embodiment at least one of the residues R¹ to R⁴ is selected from the group consisting of 2-hydroxyethyl, hydroxyprop-1-yl, hydroxyprop-2-yl, 2-hydroxybutyl or 2-hydroxy-2-phenylethyl.

In one embodiment R⁵ is a polyolefin-homo- or copolymer, preferably a polypropylene, polybutene or polyisobutene residue, with a number-average molecular weight (Mₙ) of 85 to 20000, for example 113 to 10 000, or 200 to 10000 or 350 to 5000, for example 350 to 3000, 500 to 2500, 700 to 2500, or 800 to 1500. Preferred are polypropenyl, polybutenyl and polyisobutenyl radicals, for example with a number-average molecular weight Mₙ of 3500 to 5000, 350 to 3000, 500 to 2500, 700 to 2500 and 800 to 1500 g/mol.

Preferred examples of anions A⁻ are the anions of acetic acid, propionic acid, butyric acid, 2-ethylhexanoic acid, trimethylhexanoic acid, 2-propylheptanoic acid, isononanoic acid, versatic acids, decanoic acid, undecanoic acid, dodecanoic acid, saturated or unsaturated fatty acids with 12 to 24 carbon atoms, or mixtures thereof, salicylic acid, oxalic acid mono-C₁-C₄-alkyl ester, phthalic acid mono-C₁-C₄-alkyl ester, C₁₂-C₁₀₀-alkyl- and -alkenyl succinic acid, especially dodecenyl succinic acid, hexadecenyl succinic acid, eicosenyl succinic acid, and polyisobutenyl succinic acid. Further examples are methyl carbonate, ethyl carbonate, n-butyl carbonate, 2-hydroxyethyl carbonate, and 2-hydroxypropyl carbonate.

In one preferred embodiment the nitrogen compounds quaternized in the presence of an acid or in an acid-free manner are obtainable by addition of a compound which comprises at least one oxygen- or nitrogen-containing group reactive with an anhydride and additionally at least one quaternizable amino group onto a polycarboxylic anhydride compound and subsequent quaternization, especially with an epoxide, e.g. styrene or propylene oxide, in the absence of free acid, as described in WO 2012/004300, or with a carboxylic ester, e.g. dimethyl oxalate or methyl salicylate. Suitable compounds having at least one oxygen- or nitrogen-containing group reactive with anhydride and additionally at least one quaternizable amino group are especially polyamines having at least one primary or secondary amino group and at least one tertiary amino group, especially N,N-dimethyl-1,3-propane diamine, N,N-dimethyl-1,2-ethane diamine or N,N, N'-trimethyl-1,2-ethane diamine. Useful polycarboxylic anhydrides are especially dicarboxylic acids such as succinic acid, having a relatively long-chain hydrocarbyl substituent, preferably having a number-average molecular weight Mₙ for the hydrocarbyl substituent of 200 to 10.000, in particular of 350 to 5000. Such a quaternized nitrogen compound is, for example, the reaction product, obtained at 40°C, of polyisobutenylsuccinic anhydride, in which the polyisobutenyl radical typically has an Mₙ of 1000, with 3-(dimethylamino)propylamine, which constitutes a polyisobutenylsuccinic monoamide and which is subsequently quaternized with dimethyl oxalate or methyl salicylate or with styrene oxide or propylene oxide in the absence of free acid.

Further quaternized nitrogen compounds suitable as compounds are described in
WO 2006/135881 A1, page 5, line 13 to page 12, line 14;
WO 10/132259 A1, page 3, line 28 to page 10, line 25;
WO 2008/060888 A2, page 6, line 15 to page 14, line 29;
WO 2011/095819 A1, page 4, line 5 to page 9, line 29;
GB 2496514 A, paragraph [00012] to paragraph [00041];
WO 2013/117616 A1, page 3, line 34 to page 11, line 2;
WO 14/202425 A2, page 3, line 14 to page 5, line 9;
WO 14/195464 A1, page 15, line 31 to page 45, line 26 and page 75, lines 1 to 4;
WO 15/040147 A1, page 4, line 34 to page 5, line 18 and page 19, line 11 to page 50, line 10;
WO 14/064151 A1, page 5, line 14 to page 6, line 17 and page 16, line 10 to page 18, line 12;
WO 2013/064689 A1, page 18, line 16 to page 29, line 8; and
WO 2013/087701 A1, page 13, line 25 to page 19, line 30,
WO 13/000997 A1, page 17, line 4 to page 25, line 3,
WO 12/004300, page 5, lines 20 to 30, page 8, line 1 to page 10, line 10, and page 19, line 29 to page 28, line 3,
each of which is incorporated herein by reference.

In one embodiment the quaternized ammonium compound is of formula wherein in this formula
PIB stands for a polyisobutenyl residue having a number average molecular weight Mₙ of from 550 to 2300, preferably from 650 to 1500 and more preferably from 750 to 1300 g/mol,
R stands for an C₁- to C₄-alkyl or hydroxy-C₁- to C₄-alkyl, preferably methyl or 2-hydroxypropyl, and
A⁻ stands for an anion, preferably carboxylate R⁵COO⁻ or a carbonate R⁵O-COO⁻ as defined above, more preferably acetate, salicylate or methyloxalate.

In another preferred embodiment the quaternized ammonium compound is of formula wherein in this formula
PIB stands for a polyisobutenyl residue having a number average molecular weight Mₙ of from 550 to 2300, preferably from 650 to 1500 and more preferably from 750 to 1300 g/mol,
R stands for a hydroxy-C₁- to C₄-alkyl, preferably 2-hydroxypropyl.

In another embodiment the quaternized compound is of formula wherein in this formula
PIB stands for a polyisobutenyl residue having a number average molecular weight Mₙ of from 550 to 2300, preferably from 650 to 1500 and more preferably from 750 to 1300 g/mol,
R stands for an C₁- to C₄-alkyl or hydroxy-C₁- to C₄-alkyl, preferably methyl, and
A⁻ stands for an anion, preferably carboxylate R⁵COO⁻ or a carbonate R⁵O-COO⁻ as defined above, more preferably salicylate or methyloxalate.

In another embodiment the quaternized ammonium compound is of formula wherein in this formula
R^{a} stands for C₁-C₂₀-alkyl, preferably C₉- to C₁₇-alkyl, more preferably for undecyl, tridecyl, pentadecyl or heptadecyl,
R^{b} stands for a hydroxy-C₁- to C₄-alkyl, preferably 2-hydroxypropyl or 2-hydroxybutyl, and
A⁻ stands for an anion, preferably carboxylate R⁵COO⁻, as defined above, more preferably R⁵COO⁻ being a carboxylate of a fatty acid, especially A⁻ being acetate, 2-ethylhexanoate, oleate, polyisobutenyl succinate or monoesters of polyisobutenyl succinate.

In one embodiment the quaternized ammonium compound is of formula wherein in this formula
Xᵢ for i = 1 to n and 1 to m are independently of another selected from the group consisting of - CH₂-CH₂-O-, -CH₂-CH(CH₃)-O-, -CH(CH₃)-CH₂-O-, -CH₂-C(CH₃)₂-O-, -C(CH₃)₂-CH₂-O-, -CH₂-CH(C₂H₅)-O-, -CH(C₂H₅)-CH₂-O- and -CH(CH₃)-CH(CH₃)-O-, preferably selected from the group consisting of -CH₂-CH(CH₃)-O-, -CH(CH₃)-CH₂-O-, -CH₂-C(CH₃)₂-O-, -C(CH₃)₂-CH₂-O-, -CH₂-CH(C₂H₅)-O-, -CH(C₂H₅)-CH₂-O- and -CH(CH₃)-CH(CH₃)-O-, more preferably selected from the group consisting of -CH₂-CH(CH₃)-O-, -CH(CH₃)-CH₂-O-, -CH₂-C(CH₃)₂-O-, -C(CH₃)₂-CH₂-O-, - CH₂-CH(C₂H₅)-O- and -CH(C₂H₅)-CH₂-O-, most preferably selected from the group consisting of -CH₂-CH(C₂H₅)-O-, -CH(C₂H₅)-CH₂-O-, -CH₂-CH(CH₃)-O- and -CH(CH₃)-CH₂-O-, and especially selected from the group consisting of -CH₂-CH(CH₃)-O- and -CH(CH₃)-CH₂-O-,
m and n independently of another are positive integers, with the proviso that the sum (m + n) is from 2 to 50, preferably from 5 to 40, more preferably from 10 to 30, and especially from 15 to 25,
R stands for an C₁- to C₄-alkyl, preferably methyl, and
A⁻ stands for an anion, preferably carboxylate R⁵COO⁻ or a carbonate R⁵O-COO⁻ as defined above, more preferably salicylate or methyloxalate.

In another preferred embodiment the quaternized ammonium compound is of formula wherein in this formula
R^{a} and R^{b} independently of another stand for C₁-C₂₀-alkyl or hydroxy-C₁- to C₄-alkyl, preferably R^{a} stands for C₁-C₂₀-alkyl, preferably ethyl, n-butyl, n-octyl, n-dodecyl, tetradecyl or hexadecyl, and R^{b} stands for hydroxy-C₁- to C₄-alkyl, preferably 2-hydroxypropyl,
A⁻ stands for an anion, preferably carboxylate R⁵COO⁻ or a carbonate R⁵O-COO⁻ as defined above, more preferably C₁₂-C₁₀₀-alkyl- and -alkenyl succinic acid, especially dodecenyl succinic acid, hexadecenyl succinic acid, eicosenyl succinic acid, and polyisobutenyl succinic acid.

### Mannich adducts

Typical Mannich adducts are described in US 8449630 B2, preferred are Mannich adducts according to formula I of US 8449630 B2, which are incorporated by reference to the present document.

In a preferred embodiment the Mannich adducts are obtainable as described in US 8449630 B2, column 7, line 35 to column 9, line 52.

Preferably the Mannich adducts are obtainable by reaction of
- at least one hydrocarbyl-substituted phenol, preferably a phenol of formula V of US 8449630 B2, more preferably para hydrocarbyl-substituted phenol or para hydrocarbyl-substituted ortho-cresol, with
- at least one aldehyde, preferably acetaldehyde or formaldehyde, more preferably formaldehyde, and
- at least one amine according to variant 2 of US 8449630 B2, preferably selected from the group consisting of octylamine, 2-ethylhexylamine, nonylamine, decylamine, undecylamine, dodecylamine, tridecylamine, tetradecylamine, pentadecylamine, hexadecylamine, heptadecylamine, octadecylamine, nonadecylamine, eicosylamine, cyclooctylamine, cyclodecylamine di-n-butylamine, diisobutylamine, di-tert-butylamine, dipentylamine, dihexylamine, diheptylamine, dioctylamine, di(2-ethylhexylamine), dinonylamine, didecylamine, N-methylcyclohexylamine, N-ethylcyclohexylamine, dicyclohexylamine, triethylenetetramine, tetraethylenepentamine, pentaethylenehexamine, dipropylenetriamine, tripropylenetetramine, tetrapropylenepentamine, dibutylenetriamine, tributylenetetramine, tetrabutylenepentamine, N, N-dipropylmethylenediamine, N, N-dipropylethylene-1, 2-diamine, N, N-dimethylpropylene- 1, 3-diamine, N, N-diethylpropylene- 1, 3-diamine, N, N-dipropylpropylene-1, 3-diamine, N, N-diethylbutylene-1, 4-diamine, N, N-dipropylbutylene-1, 4-diamine, N, N-dimethylpentylene-1, 3-diamine, N, N-diethylpentylene- 1, 5-diamine, N, N-dipropylpentylene-1, 5-diamine, N, N-dimethylhexylene-1, 6-diamine, N, N-diethylhexylene- 1, 6-diamine, N, N-dipropylhexylene-1, 6-diamine, bis [2-(N,N-dimethylamino)ethyl] amine, bis [2-(N,N-dipropylamino)ethyl]amine, bis[3-(N, N-dimethylamino)propyl]amine, bis[3-(N, N-diethylamino)-propyl]amine, bis [3-(N,N-dipropylamino)propyl] amine, bis[4-(N, Ndimethylamino) butyl]amine, bis[4-(N, N-diethylamino) butyl]amine, bis[4-(N, N-dipropylamino)butyl]amine, bis[5-(N, N-dimethylamino)-pentyl] amine, bis[5-(N, N-diethylamino)pentyl]amine, bis[5-(N, N-dipropylamino)pentyl]amine, bis[6-(N, N-dimethylamino)-hexyl]amine, bis [6-(N,N-diethylamino)hexyl] amine, bis[6-(N, N-dipropylamino) hexyl]amine, tris[2-(N, N-dimethylamino) ethyl]amine, tris[2-(N, N-dipropylamino)ethyl]amine, tris[3-(N, N-dimethylamino)propyl] amine, tri s [3-(N,Ndiethylamino)propyl]amine, tris[3-(N, N-dipropylamino)propyl]amine, tris[4-(N, N-dimethylamino)butyl]amine, tris[4-(N,N-diethylamino)-butyl] amine, tris[4-(N, Ndipropylamino)butyl]amine, tris[5-(N, N-dimethylamino)pentyl]amine, tris[5-(N, N-diethylamino)pentyl]amine, tris[5-(N,N-dipropylamino)pentyl]amine, tris[6-(N, N-dimethylamino)hexyl]amine, tris[6-(N, N-diethylamino)-hexyl]amine, and tris[6-(N, N-dipropylamino)hexyl]amine,
more preferably selected from the group consisting of dimethylamine, diethylamine, di-n-butylamine, diethylenetriamine, triethylenetetramine, tetraethylenepentamine, pentaethylenehexamine, N, N-dimethylpropylene- 1, 3-diamine, and N, N-diethylpropylene- 1, 3-diamine.

The hydrocarbyl residue of the at least one hydrocarbyl-substituted phenol preferably has a number average molecular weight Mn of from 85 to 5000, preferably of from 113 to 2500, more preferably of from 550 to 1500, and especially from 750 to 1100.

In a preferred embodiment the hydrocarbyl residue is a polyisobutene radical of the before-mentioned molecular weight, more preferably derived from a "reactive" polyisobutene radical as defined in US 8449630 B2.

In a preferred embodiment the Mannich adduct is of formula or of formula wherein
R¹⁰ is a hydrocarbyl residue with a number average molecular weight Mn of from 85 to 5000, preferably of from 113 to 2500, more preferably of from 550 to 1500, and most preferably of from 750 to 1100, and especially is a polyisobutene radical of the before-mentioned molecular weight, more preferably derived from a "reactive" polyisobutene radical,
R¹¹ is hydrogen, methyl, ethyl, iso-propyl, n-butyl, tert-butyl, but-2-yl, or amyl, preferably hydrogen or methyl, and more preferably methyl,
R¹² and R¹³ independently of another are C₁- to C₆-alkyl, preferably C₁- to C₄-alkyl, more preferably are methyl, ethyl, n-propyl, iso-propyl, n-butyl, tert-butyl, even more preferably are methyl, ethyl or n-butyl, or R¹² and R¹³ together the nitrogen atom form a five- or six-membered ring, preferably a pyrrolidine, piperidine or morpholine ring, and
R¹⁴ is bivalent alkylene residue having 1 to 6 carbon atoms, preferably 1 to 4 carbon atoms, more preferably 2 or 3 carbon atoms, most preferably selected from the group consisting of methylene, 1,2-ethylene, 1,2-propylene, 1,3-propylene, 1,4-butylene, and 1,6-hexylene, and especially being 1,2-ethylene or 1,3-propylene.

### Polyalkenemono- or polyalkenepolyamines

Polyalkenemono- or polyalkenepolyamines are preferably based on polypropene or on high-reactivity (i.e. having predominantly terminal double bonds) or conventional (i.e. having predominantly internal double bonds) polybutene or especially polyisobutene with Mₙ = 300 to 5000, more preferably 500 to 2500 and especially 700 to 2500. Such additives based on high-reactivity polyisobutene, which can be prepared from the polyisobutene which may comprise up to 20% by weight of n-butene units by hydroformylation and reductive amination with ammonia, monoamines or polyamines such as dimethylaminopropylamine, ethylenediamine, diethylenetriamine, triethylenetetramine or tetraethylenepentamine, are known especially from EP-A 244 616. When polybutene or polyisobutene having predominantly internal double bonds (usually in the β and γ positions) are used as starting materials in the preparation of the additives, a possible preparative route is by chlorination and subsequent amination or by oxidation of the double bond with air or ozone to give the carbonyl or carboxyl compound and subsequent amination under reductive (hydrogenating) conditions. The amines used here for the amination may be, for example, ammonia, monoamines or the abovementioned polyamines. Corresponding additives based on polypropene are described more particularly in WO-A 94/24231.

Further particular additives comprising monoamino groups are the hydrogenation products of the reaction products of polyisobutenes having an average degree of polymerization P = 5 to 100 with nitrogen oxides or mixtures of nitrogen oxides and oxygen, as described more particularly in WO-A 97/03946.

Further particular additives comprising monoamino groups are the compounds obtainable from polyisobutene epoxides by reaction with amines and subsequent dehydration and reduction of the amino alcohols, as described more particularly in DE-A 196 20 262.

Examples of particularly useful polyalkylene radicals are polyisobutenyl radicals derived from what are called "high-reactivity" polyisobutenes which feature a high content of terminal double bonds. Terminal double bonds are alpha-olefinic double bonds of the type which are also referred to collectively as vinylidene double bonds. Suitable high-reactivity polyisobutenes are, for example, polyisobutenes which have a proportion of vinylidene double bonds of greater than 70 mol%, especially greater than 80 mol% or greater than 85 mol%. Preference is given especially to polyisobutenes which have homogeneous polymer skeletons. Homogeneous polymer skeletons are possessed especially by those polyisobutenes formed from isobutene units to an extent of at least 85% by weight, preferably to an extent of at least 90% by weight and more preferably to an extent of at least 95% by weight. Such high-reactivity polyisobutenes preferably have a number-average molecular weight within the abovementioned range. In addition, the high-reactivity polyisobutenes may have a polydispersity in the range from 1.05 to 7, especially of about 1.1 to 2.5, for example of less than 1.9 or less than 1.5. Polydispersity is understood to mean the quotient of weight-average molecular weight Mw divided by the number-average molecular weight Mn.

Particularly suitable high-reactivity polyisobutenes are, for example, the Glissopal brands from BASF SE, especially Glissopal^{®} 1000 (Mn = 1000), Glissopal^{®} V 33 (Mn = 550) and Glissopal^{®} 2300 (Mn = 2300), and mixtures thereof. Other number-average molecular weights can be established in a manner known in principle by mixing polyisobutenes of different number-average molecular weights or by extractive enrichment of polyisobutenes of particular molecular weight ranges.

Due to their high proportion of vinylidene double bonds these polyisobutenes are especially reactive to undergo hydroformylation and subsequent amination, preferably with ammonia, to yield the corresponding polyisobutene amines, which represent a preferred embodiment of the present invention.

### Corrosion inhibitors

As corrosion inhibitors in principle all compounds known in the art for application in fuels may be used.

Suitable corrosion inhibitors are, for example, succinic esters or hemiesters, in particular with polyols, fatty acid derivatives, for example oleic esters, oligomerized fatty acids, such as dimeric fatty acid, substituted ethanolamines, and products sold under the trade name RC 4801 (Rhein Chemie Mannheim, Germany) or HiTEC 536 (Afton Corporation).

According to US 6043199 the latter is believed to be a reaction product of linear or branched alkyl or alkenyl substituted succinic anhydride with substituted amino-imidazolines resulting in what are believed to be linear or branched alkyl or alkenyl substituted succinimide or amine substituted succinimides.

In a preferred embodiment the corrosion inhibitor is selected from the group consisting of
- fatty acids or fatty acid derivatives, preferably oleic acid or its esters,
- oligomerized fatty acids, preferably dimeric fatty acid, more preferably dimeric oleic acid (CAS: 61788-89-4),
- alkyl or alkenyl substituted succinic acids, esters or hemiesters, and
- olefin-carboxylic acid copolymers (see below).

In a more preferred embodiment the corrosion inhibitor is selected from the group consisting of
- oligomerized fatty acids, preferably dimeric fatty acid, more preferably dimeric oleic acid (CAS: 61788-89-4),
- alkyl or alkenyl substituted succinic acids, esters or hemiesters, and
- olefin-carboxylic acid copolymers (see below).

### Alkyl or alkenyl substituted succinic acids, esters or hemiesters

The succinic acids, esters or hemiesters are preferably substituted with C₈- to C₁₀₀-alkyl or -alkenyl radicals.

In a preferred embodiment the succinic acids or hemiesters follow formula wherein
R²⁰ is a C₈- to C₁₀₀-alkyl or C₈- to C₁₀₀-alkenyl group, preferably C₈- to C₁₀₀-alkenyl, more preferably C₁₂- to C₉₀-alkenyl, and even more preferably C₁₆- to C₈₀-alkenyl group, and
R²¹ is hydrogen or C₁- to C₂₀-alkyl or C₂- to C₄-hydroxyalkyl, preferably hydrogen.

The underlying succinic acid anhydrides are obtainable by thermal ene reaction of C₈- to C₁₀₀-alkenes, preferably oligomers or polymers of propene, 1-butene or isobutene, with maleic anhydride. The above-mentioned corrosion inhibitors are obtainable from such anhydrides by hydrolysis or reaction with the appropriate alcohol.

### Olefin-carboxylic acid copolymers

The olefin-carboxylic acid copolymer (A) is a copolymer obtainable by
- in a first reaction step (I) copolymerizing
   (Aa) at least one ethylenically unsaturated mono- or dicarboxylic acid or derivatives thereof, preferably a dicarboxylic acid,
   (Ab) at least one α-olefin having from at least 12 up to and including 30 carbon atoms,
   (Ac) optionally at least one further aliphatic or cycloaliphatic olefin which has at least 4 carbon atoms and is different than (Ab) and
   (Ad) optionally one or more further copolymerizable monomers other than monomers (Aa), (Ab) and (Ac), selected from the group consisting of
   (Ada) vinyl esters,
   (Adb) vinyl ethers,
   (Adc) (meth)acrylic esters of alcohols having at least 5 carbon atoms,
   (Add) allyl alcohols or ethers thereof,
   (Ade) N-vinyl compounds selected from the group consisting of vinyl compounds of heterocycles containing at least one nitrogen atom, N-vinylamides or N-vinyllactams,
   (Adf) ethylenically unsaturated aromatics,
   (Adg) α,β-ethylenically unsaturated nitriles,
   (Adh) (meth)acrylamides and
   (Adi) allylamines,
   followed by
- in a second optional reaction step (II) partly or fully hydrolyzing and/or saponifying anhydride or carboxylic ester functionalities present in the copolymer obtained from (I), the second reaction step being run at least when the copolymer obtained from reaction step (I) does not comprise any free carboxylic functionalities.

### Description of the copolymer (A)

The monomer (Aa) is at least one, preferably one to three, more preferably one or two and most preferably exactly one ethylenically unsaturated, preferably α,β-ethylenically unsaturated, mono- or dicarboxylic acid(s) or derivatives thereof, preferably a dicarboxylic acid or derivatives thereof.

Derivatives are understood to mean
- the corresponding anhydrides in monomeric or else polymeric form,
- mono- or dialkyl esters, preferably mono- or di-C₁-C₄-alkyl esters, more preferably mono- or dimethyl esters or the corresponding mono- or diethyl esters, and
- mixed esters, preferably mixed esters having different C₁-C₄ alkyl components, more preferably mixed methyl ethyl esters.

Preferably, the derivatives are anhydrides in monomeric form or di-C₁-C₄-alkyl esters, more preferably anhydrides in monomeric form.

In the context of this document, C₁-C₄-alkyl is understood to mean methyl, ethyl, iso-propyl, n-propyl, n-butyl, iso-butyl, sec-butyl and *tert*-butyl, preferably methyl and ethyl, more preferably methyl.

Examples of α,β-ethylenically unsaturated mono- or dicarboxylic acids are those mono- or dicarboxylic acids or derivatives thereof in which the carboxyl group or, in the case of dicarboxylic acids, at least one carboxyl group, preferably both carboxyl groups, is/are conjugated to the ethylenically unsaturated double bond.

Examples of ethylenically unsaturated mono- or dicarboxylic acids that are not α,β-ethylenically unsaturated are cis-5-norbornene-endo-2,3-dicarboxylic anhydride, exo-3,6-epoxy-1,2,3,6-tetrahydrophthalic anhydride and cis-4-cyclohexene-1,2-dicarboxylic anhydride.

Examples of α,β-ethylenically unsaturated monocarboxylic acids are acrylic acid, methacrylic acid, crotonic acid and ethylacrylic acid, preferably acrylic acid and methacrylic acid, referred to in this document as (meth)acrylic acid for short, and more preferably acrylic acid.

Particularly preferred derivatives of α,β-ethylenically unsaturated monocarboxylic acids are methyl acrylate, ethyl acrylate, n-butyl acrylate and methyl methacrylate.

Examples of dicarboxylic acids are maleic acid, fumaric acid, itaconic acid (2-methylenebutanedioic acid), citraconic acid (2-methylmaleic acid), glutaconic acid (pent-2-ene-1,5-dicarboxylic acid), 2,3-dimethylmaleic acid, 2-methylfumaric acid, 2,3-dimethylfumaric acid, methylenemalonic acid and tetrahydrophthalic acid, preferably maleic acid and fumaric acid and more preferably maleic acid and derivatives thereof.

More particularly, monomer (Aa) is maleic anhydride.

Monomer (Ab) is at least one, preferably one to four, more preferably one to three, even more preferably one or two and most preferably exactly one α-olefin(s) having from at least 12 up to and including 30 carbon atoms. The α-olefins (Ab) preferably have at least 14, more preferably at least 16 and most preferably at least 18 carbon atoms. Preferably, the α-olefins (Ab) have up to and including 28, more preferably up to and including 26 and most preferably up to and including 24 carbon atoms.

Preferably, the α-olefins may be one or more linear or branched, preferably linear, 1-alkene.

Examples of these are 1-dodecene, 1-tridecene, 1-tetradecene, 1-pentadecene, 1-hexadecene, 1-heptadecene, 1- octadecene, 1-nonodecene, 1-eicosene, 1-docosene, 1-tetracosene, 1-hexacosene, preference being given to 1-octadecene, 1-eicosene, 1-docosene and 1-tetracosene, and mixtures thereof.

Further examples of α-olefin (Ab) are those olefins which are oligomers or polymers of C₂ to C₁₂ olefins, preferably of C₃ to C₁₀ olefins, more preferably of C₄ to C₆ olefins. Examples thereof are ethene, propene, 1-butene, 2-butene, isobutene, pentene isomers and hexene isomers, preference being given to ethene, propene, 1-butene, 2-butene and isobutene.

Named examples of α-olefins (Ab) include oligomers and polymers of propene, 1-butene, 2-butene, isobutene, and mixtures thereof, particularly oligomers and polymers of propene or isobutene or of mixtures of 1-butene and 2-butene. Among the oligomers, preference is given to the trimers, tetramers, pentamers and hexamers, and mixtures thereof.

In addition to the olefin (Ab), it is optionally possible to incorporate at least one, preferably one to four, more preferably one to three, even more preferably one or two and especially exactly one further aliphatic or cycloaliphatic olefin(s) (Ac) which has/have at least 4 carbon atoms and is/are different than (Ab) by polymerization into the inventive copolymer.

The olefins (Ac) may be olefins having a terminal (α-)double bond or those having a non-terminal double bond, preferably having an α-double bond. The olefin (Ac) preferably comprises olefins having 4 to fewer than 12 or more than 30 carbon atoms. If the olefin (Ac) is an olefin having 12 to 30 carbon atoms, this olefin (Ac) does not have an α-double bond.

Examples of aliphatic olefins (Ac) are 1-butene, 2-butene, isobutene, pentene isomers, hexene isomers, heptene isomers, octene isomers, nonene isomers, decene isomers, undecene isomers and mixtures thereof.

Examples of cycloaliphatic olefins (Ac) are cyclopentene, cyclohexene, cyclooctene, cyclode-cene, cyclododecene, α- or β-pinene and mixtures thereof, limonene and norbornene.

Further examples of olefins (Ac) are polymers having more than 30 carbon atoms of propene, 1-butene, 2-butene or isobutene or of olefin mixtures comprising the latter, preferably of isobutene or of olefin mixtures comprising the latter, more preferably having a mean molecular weight M_{w} in the range from 500 to 5000 g/mol, preferably 650 to 3000 and more preferably 800 to 1500 g/mol.

Preferably, the oligomers or polymers comprising isobutene in copolymerized form have a high content of terminal ethylenic double bonds (α-double bonds), for example at least 50 mol%, preferably at least 60 mol%, more preferably at least 70 mol% and most preferably at least 80 mol%.

For the preparation of such oligomers or polymers comprising isobutene in copolymerized form, suitable isobutene sources are either pure isobutene or isobutene-containing C4 hydrocarbon streams, for example C4 raffinates, especially "raffinate 1", C4 cuts from isobutane dehydrogenation, C4 cuts from steamcrackers and from FCC crackers (fluid catalyzed cracking), provided that they have substantially been freed of 1,3-butadiene present therein. A C4 hydrocarbon stream from an FCC refinery unit is also known as a "b/b" stream. Further suitable isobutene-containing C4 hydrocarbon streams are, for example, the product stream of a propylene-isobutane cooxidation or the product stream from a metathesis unit, which are generally used after customary purification and/or concentration. Suitable C4 hydrocarbon streams comprise generally less than 500 ppm, preferably less than 200 ppm, of butadiene. The presence of 1-butene and of cis- and trans-2-butene is substantially uncritical. Typically, the isobutene concentration in said C4 hydrocarbon streams is in the range from 40% to 60% by weight. For instance, raffinate 1 generally consists essentially of 30% to 50% by weight of isobutene, 10% to 50% by weight of 1-butene, 10% to 40% by weight of cis- and trans-2-butene and 2% to 35% by weight of butanes; in the polymerization process the unbranched butenes in the raffinate 1 are generally virtually inert, and only the isobutene is polymerized.

In a preferred embodiment, the monomer source used for polymerization is a technical C4 hydrocarbon stream having an isobutene content of 1% to 100% by weight, especially of 1% to 99% by weight, in particular of 1% to 90% by weight, more preferably of 30% to 60% by weight, especially a raffinate 1 stream, a b/b stream from an FCC refinery unit, a product stream from a propylene-isobutane cooxidation or a product stream from a metathesis unit.

Especially when a raffinate 1 stream is used as isobutene source, the use of water as the sole initiator or as further initiator has been found to be useful, particularly when polymerization is effected at temperatures of -20°C to +30°C, especially of 0°C to +20°C. At temperatures of - 20°C to +30°C, especially of 0°C to +20°C, however, it is possible to dispense with the use of an initiator when using a raffinate 1 stream as isobutene source.

Said isobutene-containing monomer mixture may comprise small amounts of contaminants such as water, carboxylic acids or mineral acids without causing any critical yield or selectivity losses. It is appropriate to the purpose to avoid accumulation of these impurities by removing such harmful substances from the isobutene-containing monomer mixture, for example, by adsorption on solid adsorbents such as activated carbon, molecular sieves or ion exchangers.

It is also possible, albeit less preferable, to convert monomer mixtures of isobutene or of the isobutene-containing hydrocarbon mixture with olefinically unsaturated monomers copolymerizable with isobutene. If monomer mixtures of isobutene with suitable comonomers are to be copolymerized, the monomer mixture comprises preferably at least 5% by weight, more preferably at least 10% by weight and especially at least 20% by weight of isobutene, and preferably at most 95% by weight, more preferably at most 90% by weight and especially at most 80% by weight of comonomers.

In a preferred embodiment, the mixture of the olefins (Ab) and optionally (Ac), averaged to their molar amounts, have at least 12 carbon atoms, preferably at least 14, more preferably at least 16 and most preferably at least 17 carbon atoms.

For example, a 2:3 mixture of docosene and tetradecene has an averaged value for the carbon atoms of 0.4 × 22 + 0.6 × 14 = 17.2.

The upper limit is less relevant and is generally not more than 60 carbon atoms, preferably not more than 55, more preferably not more than 50, even more preferably not more than 45 and especially not more than 40 carbon atoms.

The optional monomer (Ad) is at least one monomer, preferably one to three, more preferably one or two and most preferably exactly one monomer(s) selected from the group consisting of
(Ada) vinyl esters,
(Adb) vinyl ethers,
(Adc) (meth)acrylic esters of alcohols having at least 5 carbon atoms,
(Add) allyl alcohols or ethers thereof,
(Ade) N-vinyl compounds selected from the group consisting of vinyl compounds of heterocycles containing at least one nitrogen atom, N-vinylamides or N-vinyllactams,
(Adf) ethylenically unsaturated aromatics and
(Adg) α,β-ethylenically unsaturated nitriles,
(Adh) (meth)acrylamides and
(Adi) allylamines.

Examples of vinyl esters (Ada) are vinyl esters of C₂- to C₁₂-carboxylic acids, preferably vinyl acetate, vinyl propionate, vinyl butyrate, vinyl pentanoate, vinyl hexanoate, vinyl octanoate, vinyl 2-ethylhexanoate, vinyl decanoate, and vinyl esters of Versatic Acids 5 to 10, preferably vinyl esters of 2,2-dimethylpropionic acid (pivalic acid, Versatic Acid 5), 2,2-dimethylbutyric acid (neohexanoic acid, Versatic Acid 6), 2,2-dimethylpentanoic acid (neoheptanoic acid, Versatic Acid 7), 2,2-dimethylhexanoic acid (neooctanoic acid, Versatic Acid 8), 2,2-dimethylheptanoic acid (neononanoic acid, Versatic Acid 9) or 2,2-dimethyloctanoic acid (neodecanoic acid, Versatic Acid 10).

Examples of vinyl ethers (Adb) are vinyl ethers of C₁- to C₁₂-alkanols, preferably vinyl ethers of methanol, ethanol, *iso-*propanol, n-propanol, n-butanol, *iso*-butanol, sec-butanol, *tert*-butanol, n-hexanol, n-heptanol, n-octanol, n-decanol, n-dodecanol (lauryl alcohol) or 2-ethylhexanol.

Preferred (meth)acrylic esters (Adc) are (meth)acrylic esters of C₅- to C₁₂-alkanols, preferably of n-pentanol, n-hexanol, n-heptanol, n-octanol, n-decanol, n-dodecanol (lauryl alcohol), 2-ethylhexanol or 2-propylheptanol. Particular preference is given to pentyl acrylate, 2-ethylhexyl acrylate, 2-propylheptyl acrylate.

Examples of monomers (Add) are allyl alcohols and allyl ethers of C₂- to C₁₂-alkanols, preferably allyl ethers of methanol, ethanol, iso-propanol, n-propanol, n-butanol, *iso-*butanol, sec-butanol, *tert*-butanol, n-hexanol, n-heptanol, n-octanol, n-decanol, n-dodecanol (lauryl alcohol) or 2-ethylhexanol.

Examples of vinyl compounds (Ade) of heterocycles comprising at least one nitrogen atom are N-vinylpyridine, N-vinylimidazole and N-vinylmorpholine.

Preferred compounds (Ade) are N-vinylamides or N-vinyllactams.

Examples of N-vinylamides or N-vinyllactams (Ade) are N-vinylformamide, N-vinylacetamide, N-vinylpyrrolidone and N-vinylcaprolactam.

Examples of ethylenically unsaturated aromatics (Adf) are styrene and α-methylstyrene.

Examples of α,β-ethylenically unsaturated nitriles (Adg) are acrylonitrile and methacrylonitrile.

Examples of (meth)acrylamides (Adh) are acrylamide and methacrylamide.

Examples of allylamines (Adi) are allylamine, dialkylallylamine and trialkylallylammonium halides.

Preferred monomers (Ad) are (Ada), (Adb), (Adc), (Ade) and/or (Adf), more preferably (Ada), (Adb) and/or (Adc), even more preferably (Ada) and/or (Adc) and especially (Adc).

The incorporation ratio of the monomers (Aa) and (Ab) and optionally (Ac) and optionally (Ad) in the polymer obtained from reaction step (I) is generally as follows:
The molar ratio of (Aa)/((Ab) and (Ac)) (in total) is generally from 10:1 to 1:10, preferably 8:1 to 1:8, more preferably 5:1 to 1:5, even more preferably 3:1 to 1:3, particularly 2:1 to 1:2 and especially 1.5:1 to 1:1.5. In the preferred particular case of maleic anhydride as monomer (Aa), the molar incorporation ratio of maleic anhydride to monomers ((Ab) and (Ac)) (in total) is about 1:1.

The molar ratio of obligatory monomer (Ab) to monomer (Ac), if present, is generally of 1:0.05 to 10, preferably of 1:0.1 to 6, more preferably of 1:0.2 to 4, even more preferably of 1:0.3 to 2.5 and especially 1:0.5 to 1.5.

In a preferred embodiment, no optional monomer (Ac) is present in addition to monomer (Ab).

The proportion of one or more of the monomers (Ad), if present, based on the amount of the monomers (Aa), (Ab) and optionally (Ac) (in total) is generally 5 to 200 mol%, preferably 10 to 150 mol%, more preferably 15 to 100 mol%, even more preferably 20 to 50 mol% and especially 0 to 25 mol%.

In a preferred embodiment, no optional monomer (Ad) is present.

In a second reaction step (II), the anhydride or carboxylic ester functionalities present in the copolymer obtained from (I) are partly or fully hydrolyzed and/or saponified.

Reaction step (II) is obligatory in case the copolymer obtained from reaction step (I) does not comprise free carboxylic acid groups.

Hydrolization of anhydride groups is preferred over saponification of ester groups.

Preferably, 10% to 100% of the anhydride or carboxylic ester functionalities present are hydrolyzed and/or saponified, preferably at least 20%, more preferably at least 30%, even more preferably at least 50% and particularly at least 75% and especially at least 85%.

For a hydrolysis, based on the anhydride functionalities present, the amount of water that corresponds to the desired hydrolysis level is added and the copolymer obtained from (I) is heated in the presence of the added water. In general, a temperature of preferably 20 to 150°C is sufficient for the purpose, preferably 60 to 100°C. If required, the reaction can be conducted under pressure in order to prevent the escape of water. Under these reaction conditions, in general, the anhydride functionalities in the copolymer are converted selectively, whereas any carboxylic ester functionalities present in the copolymer react at least only to a minor degree, if at all.

For a saponification, the copolymer is reacted with an amount of a strong base corresponding to the desired saponification level in the presence of water.

Strong bases used may preferably be hydroxides, oxides, carbonates or hydrogencarbonates of alkali metals or alkaline earth metals.

The copolymer obtained from (I) is then heated in the presence of the added water and the strong base. In general, a temperature of preferably 20 to 130°C is sufficient for the purpose, preferably 50 to 110°C. If required, the reaction can be conducted under pressure.

It is also possible to hydrolyze the carboxylic ester functionalities with water in the presence of an acid. Acids used are preferably mineral acids, carboxylic acids, sulfonic acids or phosphorus acids having a pKa of not more than 5, more preferably not more than 4.

Examples are acetic acid, formic acid, oxalic acid, salicylic acid, substituted succinic acids, aromatically substituted or unsubstituted benzenesulfonic acids, sulfuric acid, nitric acid, hydrochloric acid or phosphoric acid; the use of acidic ion exchange resins is also conceivable.

In a preferred embodiment for anhydrides, especially maleic anhydride being monomers (Aa), such anhydride moieties are partly or fully, especially fully hydrolysed while potentially existing ester groups in the copolymer remain intact. In this case no saponification in step (II) takes place.

The copolymer obtained from (I) is then heated in the presence of the added water and the acid. In general, a temperature of preferably 40 to 200°C is sufficient for the purpose, preferably 80 to 150°C. If required, the reaction can be conducted under pressure.

Should the copolymers obtained from step (II) still comprise residues of acid anions, it may be preferable to remove these acid anions from the copolymer with the aid of an ion exchanger and preferably exchange them for hydroxide ions or carboxylate ions, more preferably hydroxide ions. This is the case especially when the acid anions present in the copolymer are halides or contain sulfur or nitrogen.

The copolymer obtained from reaction step (II) generally has a weight-average molecular weight Mw of 0.5 to 20 kDa, preferably 0.6 to 15, more preferably 0.7 to 7, even more preferably 1 to 7 and especially 1.5 to 4 kDa (determined by gel permeation chromatography with tetrahydrofuran and polystyrene as standard).

The number-average molecular weight Mn is usually from 0.5 to 10 kDa, preferably 0.6 to 5, more preferably 0.7 to 4, even more preferably 0.8 to 3 and especially 1 to 2 kDa (determined by gel permeation chromatography with tetrahydrofuran and polystyrene as standard).

The polydispersity is generally from 1 to 10, preferably from 1.1 to 8, more preferably from 1.2 to 7, even more preferably from 1.3 to 5 and especially from 1.5 to 3.

The content of acid groups in the copolymer is preferably from 1 to 8 mmol/g of copolymer, more preferably from 2 to 7.5, even more preferably from 3 to 7 mmol/g of copolymer.

In a preferred embodiment, the copolymers comprise a high proportion of adjacent carboxylic acid groups, which is determined by a measurement of adjacency. For this purpose, a sample of the copolymer is heat-treated between two Teflon films at a temperature of 290°C for a period of 30 minutes and an FTIR spectrum is recorded at a bubble-free site. The IR spectrum of Teflon is subtracted from the spectra obtained, the layer thickness is determined and the content of cyclic anhydride is determined.

In a preferred embodiment, the adjacency is at least 10%, preferably at least 15%, more preferably at least 20%, even more preferably at least 25% and especially at least 30%.

The olefin-carboxylic acid copolymer (A) is applied in the form of the free acid, i.e. COOH groups are present, or in the form of the anhydride which may be an intramolecular anhydride or an intermolecular anhydride linking two dicarboxylic acid molecules together, preferably in the form of a free acid. To a minor extent, some of the carboxylic functions may be present in salt form, e.g. as alkali or alkaline metal salts salts or as ammonium or substituted ammonium salts, depending on the pH value of the liquid phase. Preferably at least 50 % of all carboxylic acid groups are available in the form of the free acid as COOH-groups, more preferably at least 66 %, very preferably at least 75 %, even more preferably at least 85 %, and especially at least 95%. A single olefin-carboxylic acid copolymer (A) or a mixture of different olefin-carboxylic acid copolymers (A) may be used.

### Carrier oils

Carrier oils additionally used may be of mineral or synthetic nature. Suitable mineral carrier oils are fractions obtained in crude oil processing, such as brightstock or base oils having viscosities, for example, from the SN 500 - 2000 class; but also aromatic hydrocarbons, paraffinic hydrocarbons and alkoxyalkanols. Likewise useful is a fraction which is obtained in the refining of mineral oil and is known as "hydrocrack oil" (vacuum distillate cut having a boiling range of from about 360 to 500°C, obtainable from natural mineral oil which has been catalytically hydrogenated under high pressure and isomerized and also deparaffinized). Likewise suitable are mixtures of the abovementioned mineral carrier oils.

Examples of suitable synthetic carrier oils are polyolefins (polyalphaolefins or polyinternalolefins), (poly)esters, (poly)alkoxylates, polyethers, aliphatic polyetheramines, alkylphenol-started polyethers, alkylphenol-started polyetheramines and carboxylic esters of long-chain alkanols.

Examples of suitable polyolefins are olefin polymers having Mₙ = 400 to 1800, in particular based on polybutene or polyisobutene (hydrogenated or unhydrogenated).

Examples of suitable polyethers or polyetheramines are preferably compounds comprising polyoxy-C₂- to C₄-alkylene moieties obtainable by reacting C₂- to C₆₀-alkanols, C₆- to C₃₀-alkanediols, mono- or di-C₂- to C₃₀-alkylamines, C₁- to C₃₀-alkylcyclohexanols or C₁- to C₃₀-alkylphenols with 1 to 30 mol of ethylene oxide and/or propylene oxide and/or butylene oxide per hydroxyl group or amino group, and, in the case of the polyetheramines, by subsequent reductive amination with ammonia, monoamines or polyamines. Such products are described more particularly in EP-A 310 875, EP-A 356 725, EP-A 700 985 and US-A 4,877,416. For example, the polyetheramines used may be poly-C₂- to C₆-alkylene oxide amines or functional derivatives thereof. Typical examples thereof are tridecanol butoxylates or isotridecanol butoxylates, isononylphenol butoxylates and also polyisobutenol butoxylates and propoxylates, and also the corresponding reaction products with ammonia.

Examples of carboxylic esters of long-chain alkanols are more particularly esters of mono-, di- or tricarboxylic acids with long-chain alkanols or polyols, as described more particularly in DE-A 38 38 918. The mono-, di- or tricarboxylic acids used may be aliphatic or aromatic acids; particularly suitable ester alcohols or ester polyols are long-chain representatives having, for example, 6 to 24 carbon atoms. Typical representatives of the esters are adipates, phthalates, isophthalates, terephthalates and trimellitates of isooctanol, isononanol, isodecanol and isotridecanol, for example di(n- or isotridecyl) phthalate.

Further suitable carrier oil systems are described, for example, in DE-A 38 26 608, DE-A 41 42 241, DE-A 43 09 074, EP-A 452 328 and EP-A 548 617.

Examples of particularly suitable synthetic carrier oils are alcohol-started polyethers having about 5 to 35, preferably about 5 to 30, more preferably 10 to 30 and especially 15 to 30 C₃- to C₆-alkylene oxide units, for example propylene oxide, n-butylene oxide and isobutylene oxide units, or mixtures thereof, per alcohol molecule. Nonlimiting examples of suitable starter alcohols are long-chain alkanols or phenols substituted by long-chain alkyl in which the long-chain alkyl radical is especially a straight-chain or branched C₆- to C₁₈-alkyl radical. Particular examples include tridecanol, heptadecanol and nonylphenol. Particularly preferred alcohol-started polyethers are the reaction products (polyetherification products) of monohydric aliphatic C₆- to C₁₈-alcohols with C₃- to C₆-alkylene oxides. Examples of monohydric aliphatic C₆-C₁₈-alcohols are hexanol, heptanol, octanol, 2-ethylhexanol, nonyl alcohol, decanol, 3-propylheptanol, undecanol, dodecanol, tridecanol, tetradecanol, pentadecanol, hexadecanol, heptadecanol, octadecanol and the constitutional and positional isomers thereof. The alcohols can be used either in the form of the pure isomers or in the form of technical grade mixtures. A particularly preferred alcohol is tridecanol. Examples of C₃- to C₆-alkylene oxides are propylene oxide, such as 1,2-propylene oxide, butylene oxide, such as 1,2-butylene oxide, 2,3-butylene oxide, isobutylene oxide or tetrahydrofuran, pentylene oxide and hexylene oxide. Particular preference among these is given to C₃- to C₄-alkylene oxides, i.e. propylene oxide such as 1,2-propylene oxide and butylene oxide such as 1,2-butylene oxide, 2,3-butylene oxide and isobutylene oxide. Especially butylene oxide is used.

Further suitable synthetic carrier oils are alkoxylated alkylphenols, as described in DE-A 10 102 913.

Particular carrier oils are synthetic carrier oils, particular preference being given to the above-described alcohol-started polyethers.

### Other additives

Typical other additives in the additive packages or fuels according to the invention may be friction modifier, dehazers, antioxidants, metal deactivators, and solvents for the packages.

### Friction modifier

Suitable friction modifiers are based typically on fatty acids or fatty acid esters. Typical examples are tall oil fatty acid, as described, for example, in WO 98/004656, and glyceryl monooleate. The reaction products, described in US 6743266 B2, of natural or synthetic oils, for example triglycerides, and alkanolamines are also suitable as such friction modifier.

Preferred lubricity improvers are described in WO 15/059063 and WO 10/005720. Furthermore, hydroxyl group-substituted tertiary amines as disclosed in WO 2014/23853 are preferred as friction modifiers.

### Dehazer

Suitable dehazer are, for example, the alkali metal or alkaline earth metal salts of alkylsubstituted phenol- and naphthalenesulfonates and the alkali metal or alkaline earth metal salts of fatty acids, and also neutral compounds such as alcohol alkoxylates, e.g. alcohol ethoxylates, phenol alkoxylates, e.g. tert-butylphenol ethoxylate or tert-pentylphenol ethoxylate, fatty acids, alkylphenols, condensation products of ethylene oxide (EO) and propylene oxide (PO), for example including in the form of EO/PO block copolymers, polyethyleneimines or else polysiloxanes.

Further suitable dehazers are EO/PO-based alkoxylates of alkylphenol-formaldehyde condensates (Novolac, resol or calixarene type), EO/PO-based alkoxylates of diols (e.g. propandiol, ethylene glycole), triols (e.g. glycerol or trimethylolpropane), ethylene diamine, or polyethyleneimine. Further suitable dehazers are alkybenzene sulfonic acids, dialkylsulfosuccinates or alkali metal or ammonium salts thereof. Suitable dehazers are described in WO 96/22343. Further suitable dehazers based on diglycidyl ethers are described in US 3383326 and US 3511882.

Other suitable dehazers are, for example, alkoxylated phenol-formaldehyde condensates, for example the products available under the trade names NALCO 7D07 (Nalco) and TOLAD 2683 (Petrolite).

### Antioxidants

Suitable antioxidants are, for example, substituted phenols, such as 2,6-di-tert-butylphenol, 2,6-di-tert-butyl-4-methyl phenol, 2,4-di-tert-butyl-6-methylphenol, preferably hindered phenols with an ester group bearing radical in paraposition, such as 3-[3,5-bis-(dimethylethyl)-4-hydroxyphenyl] propanoic acid C₆- to C₂₀-alkyl esters, e.g. 2-ethylhexyl- or stearylester, and also phenylenediamines such as N,N'-di-sec-butyl-p-phenylenediamine.

### Metal deactivators

Suitable metal deactivators are, for example, salicylic acid derivatives such as N,N'-disalicylidene-1,2-propanediamine.

### Solvents

Suitable solvents are, for example, nonpolar organic solvents such as aromatic and aliphatic hydrocarbons, for example toluene, xylenes, white spirit and products sold under the trade names SHELLSOL (Royal Dutch/Shell Group) and EXXSOL (ExxonMobil), and also polar organic solvents, for example, alcohols such as 2-ethylhexanol, 2-propylheptanol, decanol, isotridecanol and isoheptadecanol. Such solvents are usually added to the fuel together with the aforementioned additives and coadditives, which they are intended to dissolve or dilute for better handling.

Therefore, another object of the present invention is a fuel additive package for gasoline fuels, comprising
- at least one branched primary alkyl amine, the alkyl group having from 8 to 22, preferably from 10 to 17, more preferably 13 carbon atoms and with a branching of at least 1.0, preferably of from 1.0 to 8.0, more preferably from 1.5 to 7.0,
- at least one deposit control agent selected from the group consisting of
   -- quaternary ammonium compounds,
   -- Mannich adducts, and
   -- polyalkenemono- or polyalkenepolyamines having a number average molecular weight in the range 300 to 5000, and
- optionally at least one further gasoline fuel additive, selected from the group consisting of
   -- friction modifiers
   -- dehazers
   -- antioxidants
   -- metal deactivators
   -- corrosion inhibitors,
   -- carrier oils, and
   -- solvents.

Preferably the at least one further gasoline fuel additive is selected from the group consisting of corrosion inhbitors, carrier oils, and solvents.

It is an advantage of the present invention that the amount of solvents in the additive packages can be reduced by the use of the branched alkyl amines compared to the use of linear alkyl amines.

### Fuels

In the context of the present invention, gasoline fuels mean liquid hydrocarbon distillate fuels boiling in the gasoline range. It is in principle suitable for use in all types of gasoline, including "light" and "severe" gasoline species. The gasoline fuels may also contain amounts of other fuels such as, for example, ethanol.

Typically, gasoline fuels, which may be used according to the present invention exhibit, in addition, one or more of the following features:
The aromatics content of the gasoline fuel is preferably not more than 50 volume % and more preferably not more than 35 volume %. Preferred ranges for the aromatics content are from 1 to 45 volume % and particularly from 5 to 35 volume %.

The sulfur content of the gasoline fuel is preferably not more than 100 ppm by weight and more preferably not more than 10 ppm by weight. Preferred ranges for the sulfur content are from 0.5 to 150 ppm by weight and particularly from 1 to 10 ppm by weight.

The gasoline fuel has an olefin content of not more than 21 volume %, preferably not more than 18 volume %, and more preferably not more than 10 volume %. Preferred ranges for the olefin content are from 0.1 to 21 volume % and particularly from 2 to 18 volume %.

The gasoline fuel has a benzene content of not more than 1.0 volume % and preferably not more than 0.9 volume %. Preferred ranges for the benzene content are from 0 to 1.0 volume % and preferably from 0.05 to 0.9 volume %.

The gasoline fuel has an oxygen content of not more than 45 weight %, preferably from 0 to 45 weight %, and most preferably from 0.1 to 3.7 weight % (first type) or most preferably from 3.7 to 45 weight % (second type). The gasoline fuel of the second type mentioned above is a mixture of lower alcohols such as methanol or especially ethanol, which derive preferably from natural source like plants, with mineral oil based gasoline, i.e. usual gasoline produced from crude oil. An example for such gasoline is "E 85", a mixture of 85 volume % of ethanol with 15 volume % of mineral oil based gasoline. Also a fuel containing 100 % of a lower alcohol, especially ethanol, is suitable.

The amount of alcohols and ethers contained in the gasoline may vary over wide ranges. Typical maximum contents are e.g. methanol 15% by volume, ethanol 85% by volume, isopropanol 20% by volume, tert-butanol 15% by volume, isobutanol 20% by volume and ethers containing 5 or more carbon atoms in the molecule 30% by volume.

The summer vapor pressure of the gasoline fuel is usually not more than 70 kPa and preferably not more than 60 kPa (at 37°C).

The research octane number ("RON") of the gasoline fuel is usually from 90 to 100. A usual range for the corresponding motor octane number ("MON") is from 80 to 90.

The above characteristics are determined by conventional methods (DIN EN 228).

Therefore, another object of the present invention is an unleaded gasoline composition suitable for use in a spark ignition engine for reducing injector nozzle fouling in a direct injection spark ignition engine, comprising
- 10 to 3000 ppmw based on the gasoline composition of a branched primary alkyl amine R-NH₂, the alkyl group R having from 8 to 22, preferably from 10 to 17, more preferably 13 carbon atoms and with a branching of at least 1.0 determined by ¹H-NMR spectroscopy, preferably from 1.0 to 8.0, more preferably from 1.5 to 7.0, wherein the amine group is bound to a primary carbon forming a group -CH₂-NH₂.

Another object of the present invention is an unleaded gasoline composition suitable for use in a spark ignition engine for reducing injector nozzle fouling in a direct injection spark ignition engine, comprising
- 10 to 3000 ppmw based on the gasoline composition of a branched primary alkyl amine R-NH₂, the alkyl group R having from 8 to 22, preferably from 10 to 17, more preferably 13 carbon atoms and with a branching of at least 1.0 determined by ¹H-NMR spectroscopy, preferably from 1.0 to 8.0, more preferably from 1.5 to 7.0 further comprising at least one deposit control agent selected from the group consisting of
- from 10 to 100 ppm by weight quaternary ammonium compounds,
- 10 to 1000 ppm by weight Mannich adducts, and
- 10 to 1000 ppm by weight polyalkenemono- or polyalkenepolyamines having a number average molecular weight in the range 300 to 5000.

Another object of the present invention is a fuel additive package for unleaded gasoline fuels for reducing injector nozzle fouling in a direct injection spark ignition engine, comprising
- at least one branched primary alkyl amine R-NH₂, the alkyl group R having from 8 to 22, preferably from 10 to 17, more preferably 13 carbon atoms and with a branching of at least 1.0 determined by ¹H-NMR spectroscopy, preferably of from 1.0 to 8.0, more preferably from 1.5 to 7.0,
- at least one deposit control agent selected from the group consisting of
   -- quaternary ammonium compounds,
   -- Mannich adducts, and
   -- polyalkenemono- or polyalkenepolyamines having a number average molecular weight in the range 300 to 5000, and
- optionally at least one further gasoline fuel additive, selected from the group consisting of
   -- corrosion inhibitors,
   -- carrier oils, and
   -- solvents.

Preferably the at least one further unleaded gasoline fuel additive is selected from the group consisting of corrosion inhbitors, carrier oils, and solvents.

The unleaded gasoline fuels according to the present invention comprise said at least one branched alkyl amine in an amount of from 10 to 3000 ppm, preferably from 15 to 1000 ppm, more preferably from 20 to 500 ppm, most preferably from 25 to 250 ppm.

The deposit control agent or mixture of a plurality of such additives is present in the unleaded gasoline fuels in the case of polyalkenemono- or polyalkenepolyamines or Mannich adducts typically in an amount of from 10 to 1000 ppm by weight, preferably of from 25 to 500 ppm by weight, more preferably of from 50 to 250 ppm by weight (based on the gasoline composition).

In the case of quaternary ammonium compounds as deposit control agents they are typically present in the unleaded gasoline fuels in an amount of from 10 to 100 ppm by weight, preferably of from 20 to 50 ppm by weight (based on the gasoline composition).

The one or more corrosion inhibitors, if any, are present in the unleaded gasoline fuels normally in an amount of from 0.1 to 10 ppm by weight, preferably of from 0.2 to 8 ppm by weight, more preferably of from 0.3 to 7 ppm by weight, most preferably of from 0.5 to 5 ppm by weight, for example of from 1 to 3 ppm by weight.

The one or more carrier oils, if any, are present in the unleaded gasoline fuels normally in an amount of form 10 to 3.000 ppm by weight, preferably of from 20 to 1000 ppm by weight, more preferably of from 50 to 700 ppm by weight, most preferably of from 70 to 500 ppm by weight.

One or more dehazers as additive component, if any, are present in the unleaded gasoline fuels generally in an amount of from 0.5 to 100 ppm by weight, preferably of from 1 to 50 ppm by weight, more preferably of from 1.5 to 40 ppm by weight, most preferably of from 2 to 30 ppm by weight, for example of from 3 to 20 ppm by weight.

The other additive components described above each, if any, are present in the unleaded gasoline fuels generally in an amount of from 0.5 to 200 ppm by weight, preferably of from 1 to 100 ppm by weight, more preferably of from 1.5 to 40 ppm by weight, most preferably of from 2 to 30 ppm by weight.

Subject matter of the present invention is also a fuel additive concentrate suitable for use in unleaded gasoline fuels comprising
0.01 to 40% by weight, preferably 0.05 to 20% by weight, more preferably 0.1 to 10% by weight, of the at least one branched alkyl amine;
10 to 70% by weight, preferably 15 to 60% by weight, more preferably 20 to 50% by weight, of the at least one deposit control agent;
0.25 to 5% by weight, preferably 0.5 to 5 by weight, more preferably 0.75 to 3.5% by weight, most preferably 1.0 to 2% by weight, of at least one corrosion inhibitor;
0 to 80% by weight, preferably 5 to 60% by weight, more preferably 10 to 40% by weight, of at least one carrier oil;
0 to 80% by weight, preferably 5 to 50% by weight, more preferably 10 to 40% by weight, of at least one solvent or diluent; and
0 to 15% by weight, preferably 0.5 to 10 by weight, more preferably 1 to 8% by weight, most preferably 3 to 7% by weight, of each of the other additive components described above, if any; with the proviso that the sum of components always results in 100%.

The amounts given throughout the text refer to the pure components excluding e.g. solvent, unless stated otherwise.

### Examples

### Example 1: Determination of injector cleanliness with a direct injection spark ignition engine.

### 1. Injector cleanliness in direct injecting gasoline engines (Direct Injection Spark Ignition (DISI) or Gasoline Direct Injection (GDI)): Keep-clean performance

The test method is a preliminary version of the upcoming CEC test for injector fouling in DISI engines (TDG-F-113) and was published by D. Weissenberger, J. Pilbeam, "Characterisation of Gasoline Fuels in a DISI Engine", lecture held at Technische Akademie Esslingen, June 27, 2017. The test engine is a VW EA111 1.4L TSI engine with 125 kW. The test procedure is a steady state test at an engine speed of 2000 rpm and a constant torque of 56 Nm.

The test procedure is performed with the following injectors: Magneti Marelli 03C 906 036 E. Reference oil RL-271 from Haltermann Carless was used as engine oil.

### 2. Injector cleanliness in direct injecting gasoline engines (Direct Injection Spark Ignition (DISI) or Gasoline Direct Injection (GDI)): Clean-up performance

In the dirty-up-clean-up sequence dirty-up is achieved by running the engine over 48 hours as described for the keep-clean procedure (see above) with base fuel. The relative change of activation time is determined as described above for the keep-clean test. The subsequent clean-up run is done with additized base fuel over 10 h. At the end of the test 3 data points are determined within 15 minutes, which mean value gives the activation time at end of clean-up test. The test result for the clean-up is the relative change of activation time of the injectors relative to the aver-age activation time determined at the end of the dirty-up phase

The test was run with an EN 228 compliant low sulfur Haltermann DISI TSI fuel according to CEC RF-83 mod complying with EN 228.

The dirty-up phase used fuel without additive and was run for 48 hours, the clean-up phase using additized fuel for 10 hours.

In Run 1 the fuel contained 300 mg/kg PIBA* and 30 mg/kg linear dodecylamin

In Run 2 the fuel contained 300 mg/kg PIBA* and 30 mg/kg branched tridecylamin obtained by amination from the corresponding tridecanol isomeric mixture with a branching index of 2.2 determined following the above-mentioned procedure.
* Kerocom(R) PIBA (65% by weight solution of polyisobutylene amine based on high-reactivity polyisobutene (after hydroformylation and amination), Mn=1000, in an aliphatic hydrocarbon mixture)

Nozzle coking is measured as change of activation time of the injector (ti_I), which is measured periodically within the test procedure. Due to nozzle coking, the hole diameters of the injector holes are reduced, and the activation time adjusted by the Engine Control Unit (ECU) accordingly. The activation time in milliseconds is a direct readout from the ECU via ECU control software. A prolongation of activation time is an indicator for nozzle coking. The test duration was 48 h.

After a run-in period of 30 minutes 3 data points for ti_I were determined within 15 minutes, which mean value gives the activation time at start of test. At the end of the test 3 data points were determined within 15 minutes, which mean value gives the activation time at end of test. The test result is the relative change of activation time ti_I of the injectors.

| | | | |
|---|---|---|---|
| Run 1 (for comparison) | dirty-up: | 14.14% | clean-up: 92.3% |
| Run 2 (according to the invention) | dirty-up: | 11.32% | clean-up: 104.25% |

It can easily be seen that the additive package comprising the branched alkyl amine according to the invention shows at least the same activity in reducing injector nozzle fouling as the linear dodecyl amine according to the prior art, if not even an improved activity.

### Example 2: Determination of storage stability of a fully formulated gasoline additive package

Three gasoline performance packages were formulated according to the following table. The carrier fluid used is a propoxylated tridecanol derived from trimerbutene (after hydroformylation and hydrogenation). Clear formulations were obtained in both cases.

| | Formulation 1 [wt%] | Formulation 2 [wt%] (Comparative) | Formulation 3 [wt%] (Comparative) |
|---|---|---|---|
| Kerocom PIBA* | 38.01 | 38.01 | 31.35 |
| Carrier fluid** | 13.37 | 13.37 | 11.03 |
| Corrosion inhibitor*** | 0.85 | 0.85 | 0.7 |
| branched tridecylamin | 5.31 | -- | -- |
| linear dodecylamin | -- | 5.31 | 4.38 |
| Solvent Naphtha heavy**** | 42.46 | 42.46 | 52.54 |
| Sum | 100 | 100 | 100 |

| | | | |
|---|---|---|---|
| * Kerocom(R) PIBA (65% by weight solution of polyisobutylene amine based on high-reactivity polyisobutene (after hydroformylation and amination), Mn=1000, in an aliphatic hydrocarbon mixture) ** propoxylated tridecanol derived from trimerbutene (after hydroformylation and hydrogenation) *** copolymer of maleic anhydride and C₂₀- to C₂₄-olefin according to synthetic example 2 of WO 15/114029 **** solvent | | | |

All three formulations were stored at 40°C, room temperature and -20 °C for one week to evaluate their storage stability.

| | Formulation 1 | Formulation 2 (Comparative) | Formulation 3 (Comparative) |
|---|---|---|---|
| +40 °C | liquid, homogeneous | liquid, homogeneous | liquid, homogeneous |
| Room temperature | liquid, homogeneous | sediment | liquid, homogeneous |
| -20 °C | liquid, homogeneous | nearly solid | liquid, homogeneous |

It can easily be seen that Comparative Formulation 2 using the same weight composition of the components as Formulation 1 according to the invention exhibits a much worse storage stability than Formulation 1.

In order to yield a comparable storage stability the amount of solvent has to be significantly increased (Comparative Formulation 3).

## Claims

1. Use of branched primary alkyl amine R-NH₂, the alkyl group R having from 8 to 22, preferably from 10 to 17, more preferably 13 carbon atoms and with a branching of at least 1.0 determined by ¹H-NMR spectroscopy, preferably of from 1.0 to 8.0, more preferably from 1.5 to 7.0 as a fuel additive in an unleaded gasoline composition suitable for use in a spark ignition engine, for reducing injector nozzle fouling in a direct injection spark ignition engine.

2. Use of branched primary alkyl amine R-NH₂, the alkyl group R having from 8 to 22, preferably from 10 to 17, more preferably 13 carbon atoms and with a branching of at least 1.0 determined by ¹H-NMR spectroscopy, preferably of from 1.0 to 8.0, more preferably from 1.5 to 7.0 as an additive in a fuel additive package for improving the storage stability and/or formulability of fuel additive packages comprising
- at least one deposit control agent selected from the group consisting of
-- quaternary ammonium compounds,
-- Mannich adducts, and
-- polyalkenemono- or polyalkenepolyamines having a number average molecular weight in the range 300 to 5000, and
- optionally at least one further gasoline fuel additive, selected from the group consisting of
-- friction modifiers
-- dehazers
-- antioxidants
-- metal deactivators
-- corrosion inhibitors,
-- carrier oils, and
-- solvents
for unleaded gasoline compositions suitable for use in a spark ignition engine, for reducing injector nozzle fouling in a direct injection spark ignition engine.

3. Use according to claim 1, wherein the gasoline composition further comprises at least one deposit control agent selected from the group consisting of
- quaternary ammonium compounds,
- Mannich adducts, and
- polyalkenemono- or polyalkenepolyamines having a number average molecular weight in the range 300 to 5000.

4. Use according to any of the preceding claims, wherein the branched primary alkyl amine is selected from the group consisting of
- 2-propyl heptyl amine,
- branched nonyl amine,
- branched tridecyl amine, and
- branched heptadecyl amine.

5. Unleaded gasoline composition suitable for use in a spark ignition engine for reducing injector nozzle fouling in a direct injection spark ignition engine, comprising
- 10 to 3000 ppmw based on the gasoline composition of a branched primary alkyl amine R-NH₂, the alkyl group R having from 8 to 22, preferably from 10 to 17, more preferably 13 carbon atoms and with a branching of at least 1.0 determined by ¹H-NMR spectroscopy, preferably from 1.0 to 8.0, more preferably from 1.5 to 7.0,
wherein the amine group is bound to a primary carbon forming a group -CH₂-NH₂.

6. Unleaded gasoline composition suitable for use in a spark ignition engine for reducing injector nozzle fouling in a direct injection spark ignition engine, comprising
- 10 to 3000 ppmw based on the gasoline composition of a branched primary alkyl amine R-NH₂, the alkyl group R having from 8 to 22, preferably from 10 to 17, more preferably 13 carbon atoms and with a branching of at least 1.0 determined by ¹H-NMR spectroscopy, preferably from 1.0 to 8.0, more preferably from 1.5 to 7.0
further comprising at least one deposit control agent selected from the group consisting of
- from 10 to 100 ppm by weight quaternary ammonium compounds,
- 10 to 1000 ppm by weight Mannich adducts, and
- 10 to 1000 ppm by weight polyalkenemono- or polyalkenepolyamines having a number average molecular weight in the range 300 to 5000.

7. Unleaded gasoline composition according to claim 6, wherein the at least one deposit control agent is of the formula
⁺NR¹R²R³R⁴ A⁻
in which
A⁻ stands for an anion, preferably a carboxylate R⁵COO⁻ or a carbonate R⁵O-COO⁻,
and
R¹, R², R³, R⁴, and R⁵ independently of another are an organic residue with from 1 to 100 carbon atoms, substituted or unsubstituted, preferably unsubstituted, linear or branched alkyl, alkenyl or hydroxyalkyl residue with 1 to 100, more preferably 1 to 75, even more preferably 1 to 30, most preferably 1 to 25 and especially 1 to 20 carbon atoms,
R⁵ additionally may be substituted or unsubstituted cycloalkyl or aryl residues bearing 5 to 20, preferably 5 to 12 carbon atoms.

8. Unleaded gasoline composition according to claim 6, wherein the at least one deposit control agent is obtainable by addition of a compound which comprises at least one oxygen- or nitrogen-containing group reactive with an anhydride and additionally at least one quaternizable amino group onto a polycarboxylic anhydride compound and subsequent quaternization in the presence of an acid or in an acid-free manner, preferably with an epoxide, especially styrene or propylene oxide, in the absence of free acid, or with a carboxylic ester, e.g. dimethyl oxalate or methyl salicylate.

9. Unleaded gasoline composition according to claim 6, wherein the at least one deposit control agent is of formula wherein in this formula
PIB stands for a polyisobutenyl residue having a number average molecular weight Mₙ of from 550 to 2300, preferably from 650 to 1500 and more preferably from 750 to 1300 g/mol,
R stands for an C₁- to C₄-alkyl or hydroxy-C₁- to C₄-alkyl, preferably methyl or 2-hydroxypropyl, and
A⁻ stands for an anion, preferably carboxylate R⁵COO⁻ or a carbonate R⁵O-COO⁻ as defined above, more preferably acetate, salicylate or methyloxalate.

10. Unleaded gasoline composition according to claim 6, wherein the at least one deposit control agent is of formula wherein in this formula
PIB stands for a polyisobutenyl residue having a number average molecular weight Mₙ of from 550 to 2300, preferably from 650 to 1500 and more preferably from 750 to 1300 g/mol,
R stands for a hydroxy-C₁- to C₄-alkyl, preferably 2-hydroxypropyl.

11. Unleaded gasoline composition according to claim 6, wherein the at least one deposit control agent is of formula wherein in this formula
PIB stands for a polyisobutenyl residue having a number average molecular weight Mₙ of from 550 to 2300, preferably from 650 to 1500 and more preferably from 750 to 1300 g/mol,
R stands for an C₁- to C₄-alkyl or hydroxy-C₁- to C₄-alkyl, preferably methyl, and
A⁻ stands for an anion, preferably carboxylate R⁵COO⁻ or a carbonate R⁵O-COO⁻ as defined above, more preferably salicylate or methyloxalate.

12. Unleaded gasoline composition according to claim 6, wherein the at least one deposit control agent is of formula wherein in this formula
R^{a} stands for C₁-C₂₀-alkyl, preferably C₉- to C₁₇-alkyl, more preferably for undecyl, tridecyl, pentadecyl or heptadecyl,
R^{b} stands for a hydroxy-C₁- to C₄-alkyl, preferably 2-hydroxypropyl or 2-hydroxybutyl, and
A⁻ stands for an anion, preferably carboxylate R⁵COO⁻, as defined above, more preferably R⁵COO⁻ being a carboxylate of a fatty acid, especially A⁻ being acetate, 2-ethylhexanoate, oleate, polyisobutenyl succinate or monoesters of polyisobutenyl succinate.

13. Unleaded gasoline composition according to claim 6, wherein the at least one deposit control agent is of formula wherein in this formula
Xᵢ for i = 1 to n and 1 to m are independently of another selected from the group consisting of -CH₂-CH₂-O-, -CH₂-CH(CH₃)-O-, -CH(CH₃)-CH₂-O-, -CH₂-C(CH₃)₂-O-, -C(CH₃)₂-CH₂-O-, -CH₂-CH(C₂H₅)-O-, -CH(C₂H₅)-CH₂-O- and -CH(CH₃)-CH(CH₃)-O-, preferably selected from the group consisting of -CH₂-CH(CH₃)-O-, -CH(CH₃)-CH₂-O-, -CH₂-C(CH₃)₂-O-, -C(CH₃)₂-CH₂-O-, -CH₂-CH(C₂H₅)-O-, -CH(C₂H₅)-CH₂-O- and -CH(CH₃)-CH(CH₃)-O-, more preferably selected from the group consisting of -CH₂-CH(CH₃)-O-,-CH(CH₃)-CH₂-O-, -CH₂-C(CH₃)₂-O-, -C(CH₃)₂-CH₂-O-, -CH₂-CH(C₂H₅)-O- and - CH(C₂H₅)-CH₂-O-, most preferably selected from the group consisting of -CH₂-CH(C₂H₅)-O-, -CH(C₂H₅)-CH₂-O-, -CH₂-CH(CH₃)-O- and -CH(CH₃)-CH₂-O-, and especially selected from the group consisting of -CH₂-CH(CH₃)-O- and -CH(CH₃)-CH₂-O-,
m and n independently of another are positive integers, with the proviso that the sum (m + n) is from 2 to 50, preferably from 5 to 40, more preferably from 10 to 30, and especially from 15 to 25,
R stands for an C₁- to C₄-alkyl, preferably methyl, and
A⁻ stands for an anion, preferably carboxylate R⁵COO⁻ or a carbonate R⁵O-COO⁻ as defined above, more preferably salicylate or methyloxalate.

14. Unleaded gasoline composition according to claim 6, wherein the at least one deposit control agent is of formula wherein in this formula
R^{a} and R^{b} independently of another stand for C₁-C₂₀-alkyl or hydroxy-C₁- to C₄-alkyl, preferably R^{a} stands for C₁-C₂₀-alkyl, preferably ethyl, n-butyl, n-octyl, n-dodecyl, tetradecyl or hexadecyl, and R^{b} stands for hydroxy-C₁- to C₄-alkyl, preferably 2-hydroxypropyl,
A⁻ stands for an anion, preferably carboxylate R⁵COO⁻ or a carbonate R⁵O-COO⁻ as defined above, more preferably C₁₂-C₁₀₀-alkyl- and -alkenyl succinic acid, especially dodecenyl succinic acid, hexadecenyl succinic acid, eicosenyl succinic acid, and polyisobutenyl succinic acid.

15. Fuel additive package for unleaded gasoline fuels for reducing injector nozzle fouling in a direct injection spark ignition engine, comprising
- at least one branched primary alkyl amine R-NH₂, the alkyl group R having from 8 to 22, preferably from 10 to 17, more preferably 13 carbon atoms and with a branching of at least 1.0 determined by ¹H-NMR spectroscopy, preferably of from 1.0 to 8.0, more preferably from 1.5 to 7.0,
- at least one deposit control agent selected from the group consisting of
-- quaternary ammonium compounds,
-- Mannich adducts, and
-- polyalkenemono- or polyalkenepolyamines having a number average molecular weight in the range 300 to 5000, and
- optionally at least one further gasoline fuel additive, selected from the group consisting of
-- corrosion inhibitors,
-- carrier oils, and
-- solvents.

## Patentansprüche

1. Verwendung von verzweigtem primärem Alkylamin R-NH₂, wobei die Alkylgruppe R 8 bis 22, vorzugsweise 10 bis 17, weiter bevorzugt 13 Kohlenstoffatome und eine durch ¹H-NMR-Spektroskopie bestimmte Verzweigung von mindestens 1,0, vorzugsweise von 1,0 bis 8,0, weiter bevorzugt von 1,5 bis 7,0, aufweist, als Kraftstoffadditiv in einer unverbleiten Benzinzusammensetzung, die zur Verwendung in einem Ottomotor geeignet ist, zur Verringerung von Ablagerungen an den Einspritzdüsen in einem direkteinspritzenden Ottomotor.

2. Verwendung von verzweigtem primärem Alkylamin R-NH₂, wobei die Alkylgruppe R 8 bis 22, vorzugsweise 10 bis 17, weiter bevorzugt 13 Kohlenstoffatome und eine durch ¹H-NMR-Spektroskopie bestimmte Verzweigung von mindestens 1,0, vorzugsweise von 1,0 bis 8,0, weiter bevorzugt von 1,5 bis 7,0, aufweist, als Additiv in einem Kraftstoffadditivpaket zur Verbesserung der Lagerstabilität und/oder Formulierbarkeit von Kraftstoffadditivpaketen, umfassend
mindestens ein Mittel zur Verhinderung von Ablagerungen, ausgewählt aus der Gruppe bestehend aus
-- quartären Ammoniumverbindungen,
-- Mannich-Addukten und
-- Polyalkenmono- oder Polyalkenpolyaminen mit einem zahlenmittleren Molekulargewicht im Bereich von 300 bis 5000 und
- gegebenenfalls mindestens einem weiteren Benzinkraftstoffadditiv, ausgewählt aus der Gruppe bestehend aus
-- Reibungsmodifikatoren,
-- Enttrübungsmitteln,
-- Antioxidantien,
-- Metalldesaktivatoren,
-- Korrosionsinhibitoren,
-- Trägerölen und
-- Lösungsmitteln,
für unverbleite Benzinzusammensetzungen, die zur Verwendung in einem Ottomotor geeignet sind, zur Verringerung von Ablagerungen an den Einspritzdüsen in einem direkteinspritzenden Ottomotor.

3. Verwendung nach Anspruch 1, wobei die Benzinzusammensetzung ferner mindestens ein Mittel zur Verhinderung von Ablagerungen umfasst, das ausgewählt ist aus der Gruppe bestehend aus
- quartären Ammoniumverbindungen,
- Mannich-Addukten und
- Polyalkenmono- oder Polyalkenpolyaminen mit einem zahlenmittleren Molekulargewicht im Bereich von 300 bis 5000.

4. Verwendung nach einem der vorhergehenden Ansprüche, wobei das verzweigte primäre Alkylamin ausgewählt ist aus der Gruppe bestehend aus
- 2-Propylheptylamin,
- verzweigtem Nonylamin,
- verzweigtem Tridecylamin und
- verzweigtem Heptadecylamin.

5. Unverbleite Benzinzusammensetzung, die zur Verwendung in einem Ottomotor geeignet ist, zur Verringerung von Ablagerungen an den Einspritzdüsen in einem direkteinspritzenden Ottomotor, umfassend
- 10 bis 3000 Gew.-ppm, bezogen auf die Benzinzusammensetzung, eines verzweigten primären Alkylamins R-NH₂, wobei die Alkylgruppe R 8 bis 22, vorzugsweise 10 bis 17, weiter bevorzugt 13 Kohlenstoffatome und eine durch ¹H-NMR-Spektroskopie bestimmte Verzweigung von mindestens 1,0, vorzugsweise von 1,0 bis 8,0, weiter bevorzugt von 1,5 bis 7,0, aufweist,
wobei die Amingruppe an einen primären Kohlenstoff gebunden ist, wodurch sich eine Gruppe -CH₂-NH₂ ergibt.

6. Unverbleite Benzinzusammensetzung, die zur Verwendung in einem Ottomotor geeignet ist, zur Verringerung von Ablagerungen an den Einspritzdüsen in einem direkteinspritzenden Ottomotor, umfassend
- 10 bis 3000 Gew.-ppm, bezogen auf die Benzinzusammensetzung, eines verzweigten primären Alkylamins R-NH₂, wobei die Alkylgruppe R 8 bis 22, vorzugsweise 10 bis 17, weiter bevorzugt 13, Kohlenstoffatome und eine durch 1H-NMR-Spektroskopie bestimmte Verzweigung von mindestens 1,0, vorzugsweise von 1,0 bis 8,0, weiter bevorzugt von 1,5 bis 7,0, aufweist,
ferner umfassend mindestens ein Mittel zur Verhinderung von Ablagerungen, ausgewählt aus der Gruppe bestehend aus
- 10 bis 100 Gew.-ppm quaternären Ammoniumverbindungen,
- 10 bis 1000 Gew.-ppm Mannich-Addukten und
- 10 bis 1000 Gew.-ppm Polyalkenmono- oder Polyalkenpolyaminen mit einem zahlenmittleren Molekulargewicht im Bereich von 300 bis 5000.

7. Unverbleite Benzinzusammensetzung nach Anspruch 6, wobei das mindestens eine Mittel zur Verhinderung von Ablagerungen die folgende Formel aufweist:
⁺NR¹R²R³R⁴ A⁻
in der
A⁻ für ein Anion, vorzugsweise ein Carboxylat R⁵COO⁻ oder ein Carbonat R⁵O-COO⁻, steht
und
R¹, R², R³, R⁴ und R⁵ unabhängig voneinander für einen organischen Rest mit 1 bis 100 Kohlenstoffatomen, der substituiert oder unsubstituiert ist, vorzugsweise einen unsubstituierten, linearen oder verzweigten Alkyl-, Alkenyl- oder Hydroxyalkylrest mit 1 bis 100, weiter bevorzugt 1 bis 75, noch weiter bevorzugt 1 bis 30, ganz besonders bevorzugt 1 bis 25 und insbesondere 1 bis 20 Kohlenstoffatomen stehen,
R⁵ zusätzlich für substituierte oder unsubstituierte Cycloalkyl- oder Arylreste mit 5 bis 20 und vorzugsweise 5 bis 12 Kohlenstoffatomen stehen kann.

8. Unverbleite Benzinzusammensetzung nach Anspruch 6, das mindestens eine Mittel zur Verhinderung von Ablagerungen erhältlich ist durch Addition einer Verbindung, die mindestens eine mit einem Anhydrid reaktive sauerstoff- oder stickstoffhaltige Gruppe und zusätzlich mindestens eine quaternisierbare Aminogruppe enthält, an eine Polycarbonsäureanhydrid-Verbindung und nachfolgende Quaternisierung in Gegenwart einer Säure oder säurefrei, vorzugsweise mit einem Epoxid, insbesondere Styrol- oder Propylenoxid, in Abwesenheit von freier Säure, oder mit einem Carbonsäureester, z. B. Dimethyloxalat oder Methylsalicylat.

9. Unverbleite Benzinzusammensetzung nach Anspruch 6, wobei das mindestens eine Mittel zur Verhinderung von Ablagerungen folgende Formel aufweist: wobei in dieser Formel
PIB für einen Polyisobutenylrest mit einem zahlenmittleren Molekulargewicht Mₙ von 550 bis 2300, vorzugsweise von 650 bis 1500 und weiter bevorzugt von 750 bis 1300 g/mol steht,
R für ein C₁- bis C₄-Alkyl oder Hydroxy-C₁- bis C₄-alkyl, vorzugsweise Methyl oder 2-Hydroxypropyl, steht und
A⁻ für ein Anion, vorzugsweise ein Carboxylat R⁵COO⁻ oder ein Carbonat R⁵O-COO⁻ gemäß obiger Definition, weiter bevorzugt Acetat, Salicylat oder Methyloxalat, steht.

10. Unverbleite Benzinzusammensetzung nach Anspruch 6, wobei das mindestens eine Mittel zur Verhinderung von Ablagerungen folgende Formel aufweist: wobei in dieser Formel
PIB für einen Polyisobutenylrest mit einem zahlenmittleren Molekulargewicht Mₙ von 550 bis 2300, vorzugsweise von 650 bis 1500 und weiter bevorzugt von 750 bis 1300 g/mol steht,
R für ein Hydroxy-C₁- bis C₄-alkyl, vorzugsweise 2-Hydroxypropyl, steht.

11. Unverbleite Benzinzusammensetzung nach Anspruch 6, wobei das mindestens eine Mittel zur Verhinderung von Ablagerungen folgende Formel aufweist: wobei in dieser Formel
PIB für einen Polyisobutenylrest mit einem zahlenmittleren Molekulargewicht Mₙ von 550 bis 2300, vorzugsweise von 650 bis 1500 und weiter bevorzugt von 750 bis 1300 g/mol steht,
R für ein C₁- bis C₄-Alkyl oder Hydroxy-C₁- bis -C₄-alkyl, vorzugsweise Methyl, steht und
A⁻ für ein Anion, vorzugsweise ein Carboxylat R⁵COO⁻ oder ein Carbonat R⁵O-COO⁻ gemäß obiger Definition, weiter bevorzugt Salicylat oder Methyloxalat, steht.

12. Unverbleite Benzinzusammensetzung nach Anspruch 6, wobei das mindestens eine Mittel zur Verhinderung von Ablagerungen folgende Formel aufweist: wobei in dieser Formel
R^{a} für C₁-C₂₀-Alkyl, vorzugsweise C₉- bis C₁₇-Alkyl, weiter bevorzugt für Undecyl, Tridecyl, Pentadecyl oder Heptadecyl, steht,
R^{b} für ein Hydroxy-C₁- bis C₄-alkyl, vorzugsweise 2-Hydroxypropyl oder 2-Hydroxybutyl, steht und
A⁻ für ein Anion, vorzugsweise Carboxylat R⁵COO⁻, gemäß obiger Definition steht, weiter bevorzugt R⁵COO⁻ ein Carboxylat einer Fettsäure ist, insbesondere A⁻ Acetat, 2-Ethylhexanoat, Oleat, Polyisobutenylsuccinat oder Monoester von Polyisobutenylsuccinat ist.

13. Unverbleite Benzinzusammensetzung nach Anspruch 6, wobei das mindestens eine Mittel zur Verhinderung von Ablagerungen folgende Formel aufweist: wobei in dieser Formel
Xᵢ für i = 1 bis n und 1 bis m unabhängig voneinander ausgewählt sind aus der Gruppe bestehend aus -CH₂-CH₂-O-, -CH₂-CH(CH₃)-O-, -CH(CH₃)-CH₂-O-, -CH₂-C(CH₃)₂-O-, - C (CH₃)₂-CH₂-O-, -CH₂-CH(C₂H₅)-O-, -CH(C₂H₅)-CH₂-O- und - CH(CH₃)-CH(CH₃)-O-, vorzugsweise ausgewählt aus der Gruppe bestehend aus -CH₂-CH(CH₃)-O-, -CH(CH₃)-CH₂-O-, - CH₂-C(CH₃)₂-O-, -C(CH₃)₂-CH₂-O-, -CH₂-CH(C₂H₅)-O-, - CH(C₂H₅)-CH₂-O- und -CH(CH₃)-CH(CH₃)-O-, weiter bevorzugt ausgewählt aus der Gruppe bestehend aus -CH₂-CH(CH₃)-O-, -CH(CH₃)-CH₂-O-, -CH₂-C(CH₃)₂-O-, -C(CH₃)₂-CH₂-O-, -CH₂-CH(C₂H₅)-O- und -CH(C₂H₅)-CH₂-O-, ganz besonders bevorzugt ausgewählt aus der Gruppe bestehend aus -CH₂-CH(C₂H₅)-O-, -CH(C₂H₅)-CH₂-O-, -CH₂-CH(CH₃)-O- und -CH(CH₃)-CH₂-O- und insbesondere ausgewählt aus der Gruppe bestehend aus - CH₂-CH(CH₃)-O- und -CH(CH₃)-CH₂-O-,
m und n unabhängig voneinander positive ganze Zahlen sind, mit der Maßgabe, dass die Summe (m + n) 2 bis 50, vorzugsweise 5 bis 40, weiter bevorzugt 10 bis 30 und insbesondere 15 bis 25 beträgt,
R für ein C₁- bis C₄-Alkyl, vorzugsweise Methyl, steht und
A⁻ für ein Anion, vorzugsweise ein Carboxylat R⁵COO⁻ oder ein Carbonat R⁵O-COO⁻ gemäß obiger Definition, weiter bevorzugt Salicylat oder Methyloxalat, steht.

14. Unverbleite Benzinzusammensetzung nach Anspruch 6, wobei das mindestens eine Mittel zur Verhinderung von Ablagerungen folgende Formel aufweist: wobei in dieser Formel
R^{a} und R^{b} unabhängig voneinander für C₁-C₂₀-Alkyl oder Hydroxy-C₁- bis C₄-alkyl stehen, vorzugsweise R^{a} für C₁-C₂₀-Alkyl, vorzugsweise Ethyl, n-Butyl, n-Octyl, n-Dodecyl, Tetradecyl oder Hexadecyl, steht und R^{b} für Hydroxy-C₁- bis C₄-alkyl, vorzugsweise 2-Hydroxypropyl, steht,
A⁻ für ein Anion, vorzugsweise ein Carboxylat R⁵COO⁻ oder ein Carbonat R⁵O-COO⁻ gemäß obiger Definition, weiter bevorzugt C₁₂-C₁₀₀-Alkyl- und -Alkenylbernsteinsäure, insbesondere Dodecenylbernsteinsäure, Hexadecenylbernsteinsäure, Eicosenylbernsteinsäure und Polyisobutenylbernsteinsäure, steht.

15. Kraftstoffadditivpaket für unverbleite Benzinkraftstoffe zur Verringerung von Ablagerungen an den Einspritzdüsen in einem direkteinspritzenden Ottomotor, umfassend
- mindestens ein verzweigtes primäres Alkylamin R-NH₂, wobei die Alkylgruppe R 8 bis 22, vorzugsweise 10 bis 17, weiter bevorzugt 13, Kohlenstoffatome und eine durch ¹H-NMR-Spektroskopie bestimmte Verzweigung von mindestens 1,0, vorzugsweise von 1,0 bis 8,0, weiter bevorzugt von 1,5 bis 7,0, aufweist,
mindestens ein Mittel zur Verhinderung von Ablagerungen, ausgewählt aus der Gruppe bestehend aus
-- quartären Ammoniumverbindungen,
-- Mannich-Addukten und
-- Polyalkenmono- oder Polyalkenpolyaminen mit einem zahlenmittleren Molekulargewicht im Bereich von 300 bis 5000 und
- gegebenenfalls mindestens einem weiteren Benzinkraftstoffadditiv, ausgewählt aus der Gruppe bestehend aus
-- Korrosionsinhibitoren,
-- Trägerölen und
-- Lösungsmitteln.

## Revendications

1. Utilisation d'alkylamine primaire ramifiée R-NH₂, le groupe alkyle R ayant de 8 à 22, préférablement de 10 à 17, plus préférablement 13 atomes de carbone et ayant une ramification d'au moins 1,0 déterminée par spectroscopie RMN ¹H, préférablement de 1,0 à 8,0, plus préférablement de 1,5 à 7,0, comme additif pour carburant dans une composition d'essence sans plomb convenant à une utilisation dans un moteur à allumage commandé, pour réduire l'encrassement des buses d'injecteurs dans un moteur à injection directe à allumage commandé.

2. Utilisation d'alkylamine primaire ramifiée R-NH₂, le groupe alkyle R ayant de 8 à 22, préférablement de 10 à 17, plus préférablement 13 atomes de carbone et ayant une ramification d'au moins 1,0 déterminée par spectroscopie RMN ¹H, préférablement de 1,0 à 8,0, plus préférablement de 1,5 à 7,0, comme additif dans un ensemble d'additif pour carburant pour améliorer la stabilité au stockage et/ou la formulabilité d'ensembles d'additif pour carburant comprenant
- au moins un agent de régulation des dépôts choisi dans le groupe constitué par
-- composés d'ammonium quaternaire,
-- adduits de Mannich, et
-- polyalcènemono- ou polyalcènepolyamines ayant un poids moléculaire moyen en nombre dans la plage de 300 à 5 000, et
- éventuellement au moins un autre additif pour carburant d'essence, choisi dans le groupe constitué par
-- modificateurs de friction
-- agents diminuant le trouble
-- antioxydants
-- désactivateurs de métaux
-- inhibiteurs de corrosion,
-- huiles de support, et
-- solvants
pour des compositions d'essence sans plomb convenant à une utilisation dans un moteur à allumage commandé, afin de réduire l'encrassement des buses d'injecteurs dans un moteur à allumage commandé à injection directe.

3. Utilisation selon la revendication 1, dans laquelle la composition d'essence comprend en outre au moins un agent de régulation des dépôts choisi dans le groupe constitué par
- composés d'ammonium quaternaire,
- adduits de Mannich, et
- polyalcènemono- ou polyalcènepolyamines ayant un poids moléculaire moyen en nombre dans la plage de 300 à 5 000.

4. Utilisation selon l'une quelconque des revendications précédentes, dans laquelle l'alkylamine primaire ramifiée est choisie dans le groupe constitué par
- 2-propylheptylamine,
- nonylamine ramifiée,
- tridécylamine ramifiée, et
- heptadécylamine ramifiée.

5. Composition d'essence sans plomb convenant à une utilisation dans un moteur à allumage commandé pour réduire l'encrassement des buses d'injecteur dans un moteur à allumage commandé à injection directe, comprenant
- 10 à 3 000 ppm en poids, par rapport à la composition d'essence, d'une alkylamine primaire ramifiée R-NH₂, le groupe alkyle R ayant de 8 à 22, préférablement de 10 à 17, plus préférablement 13 atomes de carbone et ayant une ramification d'au moins 1,0 déterminée par spectroscopie RMN ¹H, préférablement de 1,0 à 8,0, plus préférablement de 1,5 à 7,0,
dans laquelle le groupe amine est lié à un carbone primaire formant un groupe -CH₂-NH₂.

6. Composition d'essence sans plomb convenant à une utilisation dans un moteur à allumage commandé pour réduire l'encrassement des buses d'injecteur dans un moteur à allumage commandé à injection directe, comprenant
- 10 à 3 000 ppm en poids par rapport à la composition d'essence d'une alkylamine primaire ramifiée R-NH₂, le groupe alkyle R ayant de 8 à 22, préférablement de 10 à 17, plus préférablement 13 atomes de carbone et ayant une ramification d'au moins 1,0 déterminée par spectroscopie RMN ¹H, préférablement de 1,0 à 8,0, plus préférablement de 1,5 à 7,0
comprenant en outre au moins un agent de régulation des dépôts choisi dans le groupe constitué par
- de 10 à 100 ppm en poids de composés d'ammonium quaternaire,
- 10 à 1 000 ppm en poids d'adduits de Mannich, et
- 10 à 1 000 ppm en poids de polyalcènemono- ou polyalcènepolyamines ayant un poids moléculaire moyen en nombre dans la plage de 300 à 5 000.

7. Composition d'essence sans plomb selon la revendication 6, dans laquelle l'au moins un agent de régulation des dépôts est de la formule
⁺NR¹R²R³R⁴ A⁻
dans laquelle
A⁻ représente un anion, préférablement un carboxylate R⁵COO⁻ ou un carbonate R⁵O-COO⁻,
et
R¹, R², R³, R⁴, et R⁵ indépendamment les uns des autres sont un radical organique comportant de 1 à 100 atomes de carbone, un radical alkyle, alcényle ou hydroxyalkyle substitué ou non substitué, préférablement non substitué, linéaire ou ramifié comportant 1 à 100, plus préférablement 1 à 75, encore plus préférablement 1 à 30, le plus préférablement 1 à 25 et notamment 1 à 20 atomes de carbone,
R⁵ peut de plus être des radicaux cycloalkyle ou aryle substitués ou non substitués portant 5 à 20, préférablement 5 à 12 atomes de carbone.

8. Composition d'essence sans plomb selon la revendication 6, dans laquelle l'au moins un agent de régulation des dépôts peut être obtenu par ajout d'un composé qui comprend au moins un groupe contenant de l'oxygène ou de l'azote réactif avec un anhydride et de plus au moins un groupe amino quaternisable sur un composé d'anhydride polycarboxylique et quaternisation subséquente en la présence d'un acide ou d'une manière sans acide, préférablement avec un époxyde, notamment un oxyde de styrène ou de propylène, en l'absence d'acide libre, ou avec un ester carboxylique, par exemple l'oxalate de diméthyle ou le salicylate de méthyle.

9. Composition d'essence sans plomb selon la revendication 6, dans laquelle l'au moins un agent de régulation des dépôts est de formule dans cette formule
PIB représentant un radical polyisobutényle ayant un poids moléculaire moyen en nombre Mₙ allant de 550 à 2 300, préférablement de 650 à 1 500 et plus préférablement de 750 à 1 300 g/mole,
R représentant un C₁- à C₄-alkyle ou hydroxy-C₁- à C₄-alkyle, préférablement méthyle ou 2-hydroxypropyle, et A⁻ représentant un anion, préférablement carboxylate R⁵COO⁻ ou un carbonate R⁵O-COO⁻ comme défini ci-dessus, plus préférablement acétate, salicylate ou méthyloxalate.

10. Composition d'essence sans plomb selon la revendication 6, dans laquelle l'au moins un agent de régulation des dépôts est de formule dans cette formule
PIB représentant un radical polyisobutényle ayant un poids moléculaire moyen en nombre Mₙ allant de 550 à 2 300, préférablement de 650 à 1 500 et plus préférablement de 750 à 1 300 g/mole,
R représentant un hydroxy-C₁- à C₄-alkyle, préférablement 2-hydroxypropyle.

11. Composition d'essence sans plomb selon la revendication 6, dans laquelle l'au moins un agent de régulation des dépôts est de formule dans cette formule
PIB représentant un radical polyisobutényle ayant un poids moléculaire moyen en nombre Mₙ allant de 550 à 2 300, préférablement de 650 à 1 500 et plus préférablement de 750 à 1 300 g/mole,
R représentant un C₁- à C₄-alkyle ou hydroxy-C₁- à C₄-alkyle, préférablement méthyle, et
A⁻ représentant un anion, préférablement carboxylate R⁵COO⁻ ou un carbonate R⁵O-COO⁻ comme défini ci-dessus, plus préférablement salicylate ou méthyloxalate.

12. Composition d'essence sans plomb selon la revendication 6, dans laquelle l'au moins un agent de régulation des dépôts est de formule dans cette formule
R^{a} représentant C₁-C₂₀-alkyle, préférablement C₉- à C₁₇-alkyle, plus préférablement undécyle, tridécyle, pentadécyle ou heptadécyle,
R^{b} représentant un hydroxy-C₁- à C₄-alkyle, préférablement 2-hydroxypropyle ou 2-hydroxybutyle, et
A⁻ représentant un anion, préférablement carboxylate R⁵COO⁻, comme défini ci-dessus, plus préférablement R⁵COO⁻étant un carboxylate d'un acide gras, notamment A⁻ étant acétate, 2-éthylhexanoate, oléate, poly(succinate d'isobutényle) ou monoesters de poly(succinate d'isobutényle).

13. Composition d'essence sans plomb selon la revendication 6, dans laquelle l'au moins un agent de régulation des dépôts est de formule dans cette formule
Xᵢ pour i = 1 à n et 1 à m étant indépendamment les uns des autres choisis dans le groupe constitué par -CH₂-CH₂-O-, -CH₂-CH(CH₃)-O-, -CH(CH₃)-CH₂-O-, -CH₂-C(CH₃)₂-O-, - C(CH₃)₂-CH₂-O-, -CH₂-CH(C₂H₅)-O-, -CH(C₂H₅)-CH₂-O- et - CH(CH₃)-CH(CH₃)-O-, préférablement choisis dans le groupe constitué par -CH₂-CH(CH₃)-O-, -CH(CH₃)-CH₂-O-, -CH₂-C(CH₃)₂-O-, -C(CH₃)₂-CH₂-O-, -CH₂-CH(C₂H₅)-O-, -CH(C₂H₅)-CH₂-O- et -CH(CH₃)-CH(CH₃)-O-, plus préférablement choisis dans le groupe constitué par -CH₂-CH(CH₃)-O-, - CH(CH₃)-CH₂-O-, -CH₂-C(CH₃)₂-O-, -C(CH₃)₂-CH₂-O-, -CH₂-CH(C₂H₅)-O- et -CH(C₂H₅)-CH₂-O-, le plus préférablement choisis dans le groupe constitué par -CH₂-CH(C₂H₅)-O-, - CH(C₂H₅)-CH₂-O-, -CH₂-CH(CH₃)-O- et -CH(CH₃)-CH₂-O-, et notamment choisis dans le groupe constitué par -CH₂-CH(CH₃)-O- et -CH(CH₃)-CH₂-O-,
m et n étant indépendamment l'un de l'autre des entiers positifs, à la condition que la somme (m + n) soit de 2 à 50, préférablement de 5 à 40, plus préférablement de 10 à 30, et notamment de 15 à 25,
R représentant un C₁- à C₄-alkyle, préférablement méthyle, et
A⁻ représentant un anion, préférablement carboxylate R⁵COO⁻ ou un carbonate R⁵O-COO⁻ comme défini ci-dessus, plus préférablement salicylate ou méthyloxalate.

14. Composition d'essence sans plomb selon la revendication 6, dans laquelle l'au moins un agent de régulation des dépôts est de formule dans cette formule
R^{a} et R^{b} représentant indépendamment l'un de l'autre C₁-C₂₀-alkyle ou hydroxy-C₁- à C₄-alkyle, préférablement R^{a} représentant C₁-C₂₀-alkyle, préférablement éthyle, n-butyle, n-octyle, n-dodécyle, tétradécyle ou hexadécyle, et R^{b} représentant hydroxy-C₁- à C₄-alkyle, préférablement 2-hydroxypropyle,
A⁻ représentant un anion, préférablement carboxylate R⁵COO⁻ ou un carbonate R⁵O-COO⁻ comme défini ci-dessus, plus préférablement acide C₁₂-C₁₀₀-alkyl- et - alcénylsuccinique, notamment acide dodécénylsuccinique, acide hexadécénylsuccinique, acide eicosénylsuccinique, et acide polyisobuténylsuccinique.

15. Ensemble d'additif pour carburant pour carburants d'essence sans plomb destiné à réduire l'encrassement des buses d'injecteurs dans un moteur à allumage commandé à injection directe, comprenant
- au moins une alkylamine primaire ramifiée R-NH₂, le groupe alkyle R ayant de 8 à 22, préférablement de 10 à 17, plus préférablement 13 atomes de carbone et ayant une ramification d'au moins 1,0 déterminée par spectroscopie RMN ¹H, préférablement de 1,0 à 8,0, plus préférablement de 1,5 à 7,0,
- au moins un agent de régulation des dépôts choisi dans le groupe constitué par
-- composés d'ammonium quaternaire,
-- adduits de Mannich, et
-- polyalcènemono- ou polyalcènepolyamines ayant un poids moléculaire moyen en nombre dans la plage de 300 à 5 000, et
- éventuellement au moins un autre additif pour carburant d'essence, choisi dans le groupe constitué par
-- inhibiteurs de corrosion,
-- huiles de support, et
-- solvants.
